



US007807074B2

(12) **United States Patent**  
**Luly et al.**

(10) **Patent No.:** **US 7,807,074 B2**  
(b5) **Date of Patent:** **Oct. 5, 2010**

(54) **GASEOUS DIELECTRICS WITH LOW GLOBAL WARMING POTENTIALS**

(75) Inventors: **Matthew H. Luly**, Hamburg, NY (US); **Robert G. Richard**, Hamburg, NY (US)

(73) Assignee: **Honeywell International Inc.**, Morristown, NJ (US)

(\*) Notice: Subject to any disclaimer, the term of this patent is extended or adjusted under 35 U.S.C. 154(b) by 803 days.

(21) Appl. No.: **11/637,657**

(22) Filed: **Dec. 12, 2006**

(65) **Prior Publication Data**

US 2008/0135817 A1 Jun. 12, 2008

(51) **Int. Cl.**

**H01B 3/16** (2006.01)

(52) **U.S. Cl.** ..... **252/571**; 252/67; 252/68;  
252/69

(58) **Field of Classification Search** ..... 252/67,  
252/68, 69, 571

See application file for complete search history.

(56) **References Cited**

U.S. PATENT DOCUMENTS

- 2,786,804 A \* 3/1957 Nelson ..... 203/50  
4,257,905 A 3/1981 Christophorou et al.  
4,275,260 A 6/1981 Wootton  
4,288,651 A 9/1981 Wootton  
4,440,971 A 4/1984 Harrold  
4,547,316 A 10/1985 Yamauchi  
4,816,624 A 3/1989 Perrissin et al. ..... 200/148 B  
4,871,680 A \* 10/1989 Barraud et al. ..... 436/103  
5,236,611 A 8/1993 Shiflett  
5,918,140 A \* 6/1999 Wickboldt et al. ..... 438/535  
6,886,573 B2 5/2005 Hobbs et al. ..... 134/22.1  
6,897,396 B2 5/2005 Ito et al. ..... 218/120  
2002/0135029 A1 \* 9/2002 Ping et al. ..... 257/401  
2002/0137269 A1 \* 9/2002 Ping et al. ..... 438/197  
2003/0164513 A1 \* 9/2003 Ping et al. ..... 257/288  
2005/0181621 A1 \* 8/2005 Borland et al. ..... 438/752  
2006/0060818 A1 \* 3/2006 Tempel et al. ..... 252/181.3  
2006/0133986 A1 \* 6/2006 Dukhedin-Lalla et al. ... 423/500  
2009/0211449 A1 \* 8/2009 Olschimke et al. ..... 95/233

FOREIGN PATENT DOCUMENTS

- EP 0129200 A 12/1984  
EP 1146522 X 10/2001

OTHER PUBLICATIONS

CAS Reg. No. 7647-19-0, Nov. 16, 1984.\*

Takuma, et al., "Gases as a Dielectric", pp. 195-2004, Gaseous Dielectrics X, Springer, 2004.

Lutz Niemeyer, "A Systematic Search for Insulation Gases and Their Environmental Evaluation", pp. 459-464, Gaseous Dielectrics VIII, 1998.

Christophorou, et al., "Gases for Electrical Insulation and Arc Interruption: Possible Present and Future Alternatives to Purse SF6", NIST Technical Note 1425, Nov. 1997.

Shiojiri, et al., Abstract of "Life cycle impact assessment of various treatment scenarios for sulfur hexafluoride (SF6) used as an insulating gas", Environmental Progress, 2006, 25(3), 218-227.

Shiojiri, et al., Abstract of "A Life cycle impact assessment study on sulfur hexafluoride (SF6) used as a gas insulator", 2004, American Institute of Chemical Engineers, 005E1-005E/9.

Goshima, et al., Abstract of "Estimation of cross-sectional size of gas-insulated apparatus using hybrid insulation system with SF6 substitute", Gaseous Dielectrics X, 2004, pp. 253-258.

Telfer, et al., Abstract of "A novel approach to power circuit breaker design for replacement of SF6", Centre for Intelligent Monitoring Systems, Dept. of Electrical Engineering and Electronics, 2004, 44(2), pp. 72-76.

Gustavino, et al., Abstract of "Performance of glass RPC operated in streamer mode with four-fold gas mixtures containing SF6", Nuclear Instruments & Methods in Physics Research, Section A: Accelerators, Spectrometers, Detectors, and Associated Equipment, 2004, 517(1-3), pp. 101-108.

Diaz, et al., Abstract of "Effect of the percentage of SF6 (100%-10%-5%) on the decomposition of SF6-N2 mixtures under negative dc coronas in the presence of water vapour or oxygen", Journal of Physics D: Applied Physics, 2003, 36(13), pp. 1558-1564.

Yanabu, et al., Abstract of "New concept of switchgear for replacing SF6 or gas mixture", Gaseous Dielectrics IX, 9<sup>th</sup>, 2001, pp. 497-504. Knobloch, et al., Abstract of "The comparison of arc-extinguishing capability of sulfur hexafluoride (SF6) with alternative gases in high-voltage circuit-breakers", Gaseous Dielectrics VIII, 8<sup>th</sup>, 1998, pp. 565-571.

Tioursi, et al., Abstract of "Conditioning phenomena in N2, SF6, and air", IEE Conference, 467 (High Voltage Engineering, vol. 3), 1999, pp. 3.212-3.215.

Christophorou, et al., Abstract of "SF6/N2 mixtures. Basic and HV insulation properties", IEEE Transactions on Dielectrics and Electrical Insulation, 1995, 2(5), pp. 952-1003.

Pai, et al., Abstract of "Impulse breakdown of cis-octafluorobutene/sulfur hexafluoride and cis-octafluorobutene/sulfur hexafluoride/nitrogen", Gaseous Dielectr. Proc. Int. Sump., 2<sup>nd</sup>, 1980, pp. 190-199.

Devins, J.C., Abstract of "Replacement gases for sulfur hexafluoride", IEEE Transactions on Electrical Insulation, 1980, EI-15-(2), pp. 81-86.

Devins, et al., Abstract of "Replacement gases for sulfur hexafluoride", Annual Report—Conference on Electrical Insulation and Dielectric Phenomena, 1979, pp. 398-408.

Rhodes, et al., Abstract of "Assessment of the possible use of polythene/gas dielectrics in high-voltage cables", Proc. Inst. Elec. Engrs., 1965, 112-\*), pp. 1617-1624.

Howard, et al., Abstract of "Insulation properties of compressed electronegative gases", Proc. Inst. Elec. Engrs., 1957, 104(Pt. A), pp. 123-138.

\* cited by examiner

Primary Examiner—Douglas Mc Ginty

(57) **ABSTRACT**

A dielectric gaseous compound which exhibits the following properties: a boiling point in the range between about -20° C. to about -273° C.; low ozone depleting; a GWP less than about 22,200; chemical stability, as measured by a negative standard enthalpy of formation ( $\Delta H_f < 0$ ); a toxicity level such that when the dielectric gas leaks, the effective diluted concentration does not exceed its PEL; and a dielectric strength greater than air.

## 1

GASEOUS DIELECTRICS WITH LOW  
GLOBAL WARMING POTENTIALS

## FIELD

The present disclosure relates generally to a class of gaseous dielectric compounds having low global warming potentials (GWP). In particular, such gaseous dielectric compounds exhibits the following properties: a boiling point in the range between about -20° C. to about -273° C.; low, preferably non-ozone depleting; a GWP less than about 22,200; chemical stability, as measured by a negative standard enthalpy of formation ( $\Delta H_f < 0$ ); a toxicity level such that when the dielectric gas leaks, the effective diluted concentration does not exceed its PEL, e.g., a PEL greater than about 0.3 ppm by volume (i.e., an Occupational Exposure Limit (OEL or TLV) of greater than about 0.3 ppm); and a dielectric strength greater than air. These gaseous dielectric compounds are particularly useful as insulating-gases for use with electrical equipment, such as gas-insulated circuit breakers and current-interruption equipment, gas-insulated transmission lines, gas-insulated transformers, or gas-insulated substations.

## BACKGROUND

Sulfur hexafluoride ( $SF_6$ ) has been used as a gaseous dielectric (insulator) in high voltage equipment since the 1950s. It is now known that  $SF_6$  is a potent greenhouse warming gas with one of the highest global warming potentials (GWP) known. Because of its high GWP, it is being phased out of all frivolous applications. However, there is currently no known substitute for  $SF_6$  in high voltage equipment. The electrical industry has taken steps to reduce the leak rates of equipment, monitor usage, increase recycling, and reduce emissions to the atmosphere. However, it would still be advantageous to find a substitute for  $SF_6$  in electrical dielectric applications.

The basic physical and chemical properties of  $SF_6$ , its behavior in various types of gas discharges, and its uses by the electric power industry have been broadly investigated.

In its normal state,  $SF_6$  is chemically inert, non-toxic, non-flammable, non-explosive, and thermally stable (it does not decompose in the gas phase at temperatures less than 500° C.).  $SF_6$  exhibits many properties that make it suitable for equipment utilized in the transmission and distribution of electric power. It is a strong electronegative (electron attaching) gas both at room temperature and at temperatures well above ambient, which principally accounts for its high dielectric strength and good arc-interruption properties. The breakdown voltage of  $SF_6$  is nearly three times higher than air at atmospheric pressure. Furthermore, it has good heat transfer properties and it readily reforms itself when dissociated under high gas-pressure conditions in an electrical discharge or an arc (i.e., it has a fast recovery and it is self-healing). Most of its stable decomposition byproducts do not significantly degrade its dielectric strength and are removable by filtering. It produces no polymerization, carbon, or other conductive deposits during arcing, and its is chemically compatible with most solid insulating and conducting materials used in electrical equipment at temperatures up to about 200° C.

Besides its good insulating and heat transfer properties,  $SF_6$  has a relatively high pressure when contained at room temperature. The pressure required to liquefy  $SF_6$  at 21° C. is about 2100 kPa; its boiling point is reasonably low, -63.8° C., which allows pressures of 400 kPa to 600 kPa (4 to 6 atmospheres) to be employed in  $SF_6$ -insulated equipment. It is

## 2

easily liquefied under pressure at room temperature allowing for compact storage in gas cylinders. It presents no handling problems, is readily available, and reasonably inexpensive.

$SF_6$  replaced air as a dielectric in gas insulated equipment based on characteristics such as insulation ability, boiling point, compressibility, chemical stability and non-toxicity. They have found that pure  $SF_6$ , or  $SF_6$ -nitrogen mixtures are the best gases to date.

However,  $SF_6$  has some undesirable properties: it can form highly toxic and corrosive compounds when subjected to electrical discharges (e.g.,  $S_2F_{10}$ ,  $SOF_2$ ); non-polar contaminants (e.g., air,  $CF_4$ ) are not easily removed from it; its breakdown voltage is sensitive to water vapor, conducting particles, and conductor surface roughness; and it exhibits non-ideal gas behavior at the lowest temperatures that can be encountered in the environment, i.e., in cold climatic conditions (about -50° C.),  $SF_6$  becomes partially liquefied at normal operating pressures (400 kPa to 500 kPa).  $SF_6$  is also an efficient infrared (IR) absorber and due to its chemical inertness, is not rapidly removed from the earth's atmosphere. Both of these latter properties make  $SF_6$  a potent greenhouse gas, although due to its chemical inertness (and the absence of chlorine and bromine atoms in the  $SF_6$  molecule) it is benign with regard to stratospheric ozone depletion.

That is, greenhouse gases are atmospheric gases which absorb a portion of the infrared radiation emitted by the earth and return it to earth by emitting it back. Potent greenhouse gases have strong infrared absorption in the wavelength range from approximately 7  $\mu m$  to 13  $\mu m$ . They occur both naturally in the environment (e.g.,  $H_2O$ ,  $CO_2$ ,  $CH_4$ ,  $N_2O$ ) and as man-made gases that may be released (e.g.,  $SF_6$ ; perfluorinated compound (PFC); combustion products such as  $CO_2$ , nitrogen, and sulfur oxides). The effective trapping of long-wavelength infrared radiation from the earth by the naturally occurring greenhouse gases, and its reradiation back to earth, results in an increase of the average temperature of the earth's surface. Man's impact on climate change is an environmental issue that has prompted the implementation of the Kyoto Protocol regulating the emissions of man made greenhouse gases in a number of countries.

$SF_6$  is an efficient absorber of infrared radiation, particularly at wavelengths near 10.5  $\mu m$ . Additionally, unlike most other naturally occurring green house gases (e.g.,  $CO_2$ ,  $CH_4$ ),  $SF_6$  is only slowly decomposed; therefore its contribution to global warming is expected to be cumulative and long lasting. The strong infrared absorption of  $SF_6$  and its long lifetime in the environment are the reasons for its extremely high global warming potential which for a 100-year time horizon is estimated to be approximately 22,200 times greater (per unit mass) than that of  $CO_2$ , the predominant contributor to the greenhouse effect. The concern about the presence of  $SF_6$  in the environment derives exclusively from this very high value of its potency as a greenhouse gas.

Accordingly, many in the electrical equipment industry have spent substantial time and effort seeking suitable replacement gases to reduce the use of  $SF_6$  in high voltage electrical equipment. To date, the possible replacement gases have been identified as (i) mixtures of  $SF_6$  and nitrogen for which a large amount of research results are available; (ii) gases and mixtures (e.g., pure nitrogen, low concentrations of  $SF_6$  in  $N_2$ , and  $SF_6$ -He mixtures) for which a smaller yet significant amount of data is available; and (iii) potential gases for which little experimental data is available.

Some replacements which have been proposed have higher GWPs than  $SF_6$ . For example,  $CF_3SF_5$  falls into this category.

Because of fugitive emissions in the manufacture, transportation, filling and use of such chemicals, they should be avoided.

However, the present inventors have determined that given the environmental difficulty of SF<sub>6</sub>, it is necessary to relax certain of the requirements traditionally held as important and accept as an alternative gas, compromise candidates with a lower GWP. For example, gases which are non-toxic are often inert with long atmospheric lifetimes which can yield high GWP. By accepting a somewhat more reactive gas than SF<sub>6</sub>, the GWP can be greatly reduced. It may also be necessary to accept slightly more toxic materials in order to find the best alternative in these applications. Such an increase in toxicity can be offset by reducing equipment leak rates or installing monitoring equipment. In some cases, the gases discovered by the present inventors as suitable alternatives to SF<sub>6</sub> are shown to be efficient at low levels and can be mixed with nitrogen and/or another non-toxic gas to give dielectrics with greatly reduced toxicity and acceptably low GWPs.

The unique gaseous compounds discovered by the present inventors for use as substitutes for SF<sub>6</sub> can be used in some existing electrical equipment, although they would preferably be used in specific electrical equipment optimized for them. The gaseous compounds of the present disclosure are preferably used in pure form, but can also be used as part of an azeotrope, or a mixture with an appropriate second gas, such as nitrogen, CO<sub>2</sub> or N<sub>2</sub>O.

#### SUMMARY

A dielectric gaseous compound which exhibits the following properties: a boiling point in the range between about -20° C. to about -273° C.; low, preferably non-ozone depleting; a GWP less than about 22,200; chemical stability, as measured by a negative standard enthalpy of formation (dHf<0); a toxicity level such that when the dielectric gas leaks, the effective diluted concentration does not exceed its PEL (i.e., an Occupational Exposure Limit (OEL or TLV) of at least about 0.3 ppm); and a dielectric strength greater than air.

The dielectric gaseous compound is at least one compound selected from the group consisting of:

Arsenic pentafluoride  
Arsine  
Diboron tetrafluoride  
Diborane  
Perchloric acid, 2-chloro-1,1,2,2-tetrafluoroethyl ester (9CI)  
Perchloric acid, 1,2,2-trichloro-1,2-difluoroethyl ester  
Trifluoroacetyl chloride  
trifluoromethylisocyanide (CF<sub>3</sub>-NC)  
trifluoromethyl isocyanide  
trifluoro-nitroso-ethene//Trifluor-nitroso-aethen  
Tetrafluoroethene  
3,3,4,4-tetrafluoro-3,4-dihydro-[1,2]diazete  
(Difluoramino)difluoracetonitrile  
Tetrafluorooxirane  
Trifluoroacetyl fluoride  
Perfluoromethylfluorformiat  
trifluoro-acetyl hypofluorite  
perfluoro-2-aza-1-propene  
Perfluor-2-aza-1-propen (germ.)  
N-Fluor-tetrafluor-1-aethanimin (germ.)  
3,3-difluoro-2-trifluoromethyl-oxaziridine  
bis-trifluoromethyl-diazene//hexafluoro-#cis!-azomethane  
Fluoroxypentafluoroethane  
bis-trifluoromethyl peroxide  
1,1-Bis(fluoroxy)tetrafluoroaethan

Hexafluorodimethyl sulfide  
3-fluoro-3#H!-diazirine-3-carbonitrile  
Ethyne  
1,2,2-trifluoro-aziridine  
5 Ketene  
(difluoro)vinyllboran  
(Difluor)vinyllboran (germ.)  
trifluoro-vinyl-silane  
Ethinylsilan  
10 ethyl-difluor-borane  
Ethyl-difluor-boran (germ.)  
methyl-methylen-amine  
Dimethyl ether  
vinyl-silane  
15 Dimethylsilane  
Chloroethyne  
fluoroethyne//fluoro-acetylene  
Ethanenedinitrile  
tetrafluoropropyne//1,3,3,3-tetrafluoropropyne  
20 hexafluoro-oxetane  
Trifluoro(trifluoromethyl)oxirane  
1,1,1,3,3,3-Hexafluoropropanone  
pentafluoro-propionyl fluoride//perfluoropropionyl fluoride  
Trifluoromethyl trifluorovinyl ether  
25 1-Propyne  
Cyclopropane  
Propane  
Trimethylborane  
cyanoketene  
30 butatriene  
Cyano-bis(pentafluorethyl-phosphin  
Trimethyl-1,1,2,2-tetrafluorethylsilan  
methyl diborane  
Methyldiboran (germ.)  
35 carbonyl bromide fluoride  
chloro-difluoro-nitroso-methane//Chlor-difluor-nitroso-  
methan  
chloroperoxytrifluoromethane  
carbonylchlorid-fluorid  
40 Carbonychloridfluorid (germ.)  
3,3-difluoro-3#H!-diazirine  
difluoro diazomethane  
Difluordiazomethan (germ.)  
Carbonyl fluoride  
45 Difluordioxiran  
difluoro-(3-fluoro-3#H!-diazirin-3-yl)-amine  
trifluromethylazide  
Trifluormethylazid (germ.)  
tetrafluoro-diaziridine  
50 Fluorperoxytrifluormethan  
Bis(fluoroxy)difluormethan  
Trifluormethyl-phosphonylfluorid  
Cyanogen fluoride  
Trifluormethylphosphane (germ.)  
55 Diazomethane  
formaldehyde//Formalin  
(methyl)difluoroborane  
(Methyl)difluorboran (germ.)  
Chloromethane  
60 methylphosphonous acid difluoride//difluoro-methyl-phos-  
phine  
trifluoro-methoxy-silane  
Methylhypofluorid  
Methane  
65 Methylsilane  
#Si!-bromo-#Si!,#Si!"-methanediyl-bis-silane  
#Si!-iodo-#Si!,#Si!"-methanediyl-bis-silane

Difluormethylnitrit  
 trifluoromethanol  
 Formyl fluoride  
 Cyanic acid  
 Chlorine  
 Chlorine fluoride  
 Chlorine trioxide fluoride  
 carbon oxide selenide//Kohlenoxid-selenid  
 Fluorine  
 Difluorosilane  
 Fluorine oxide  
 fluorine peroxide  
 Sulfuryl fluoride  
 sulphur difluoride  
 Phosphorus trifluoride oxide  
 Phosphorus trifluoride sulfide  
 tetrafluorophosphorane  
 Tetrafluorohydrazine  
 Sulfur tetrafluoride  
 hexafluoro disiloxane  
 Hexafluorodisiloxan (germ.)  
 Nitryl fluoride  
 Hydrogen  
 Hydrogen selenide  
 Phosphorus trihydride  
 Germanium hydride  
 Silane  
 Tin tetrahydride  
 Oxygen  
 Ozone  
 Antimony monophosphide  
 Disilicon monophosphide  
 Radon  
 Argon  
 Trifluoroborane  
 Hydrogen bromide  
 Bromopentafluoroethane  
 Chlorotrifluoroethene  
 Trifluoroacetonitrile  
 trifluoromethyl isocyanate  
 trifluoromethyl thiocarbonyl fluoride  
 Trifluormethylthiocarbonylfluorid (germ.)  
 pentafluoro-nitroso-ethane//Pentafluor-nitroso-aethan  
 (trifluoromethyl-carbonyl)-difluoro-amine  
 Hexafluoroethane  
 Bis-trifluormethyl-nitroxid  
 bis-trifluoromethyl ether  
 bis(trifluoromethyl)tellurium  
 bis(trifluoromethyl)ditelluride  
 N,N-Difluor-pentafluoraethylarnin (germ.)  
 N-Fluor-bis(trifluormethyl)-amin (germ.)  
 N-Fluor-N-trifluormethoxy-perfluormethylamin (germ.)  
 fluoroformyl cyanide  
 1-chloro-1-fluoro-ethene//1-Chlor-1-fluor-aethen//1-chloro-  
 1-fluoroethylene  
 1,1-Difluoroethene  
 #trans!-1,2-difluoro-ethene//#trans!-vinylene difluoride//  
 (E)-1,2-difluoroethylene//(E)-1,2-difluoro-ethene//  
 #trans!-vinylene fluoride  
 1,2-difluoro-ethene//#cis!-vinylene difluoride//1,2-Difluor-  
 aethen//vinylene fluoride  
 #cis!-1,2-difluoro-ethene//#cis!-vinylene difluoride//(Z)-1,  
 2-difluoroethylene//(Z)-1,2-difluoro-ethene//#cis!-vi-  
 nylene fluoride  
 1,1,1,2-Tetrafluoroethane  
 1,1,2,2-Tetrafluoroethane

Fluoroethene  
 1,1,1-Trifluoroethane  
 Ether, methyl trifluoromethyl  
 Ethene  
 5 1,1-Difluoroethane  
 Fluoroethane  
 Ethane  
 fluoro-dimethyl-borane  
 Disiloxane, 1,1,3,3-tetrafluoro-1,3-dimethyl-Trifluoroethene  
 10 trifluoroacetaldehyde//Trifluor-acetaldehyd  
 Pentafluoroethane  
 Difluoromethyl trifluoromethyl ether  
 Tris(trifluoromethyl)bismuth  
 tetrafluoropropadiene//tetrafluoro-allene//1,1,3,3-tet-  
 15 rafluoro-1,2-propadiene  
 tetrafluorocyclopropene  
 Perfluoropropionyliodid  
 pentafluoro-propionitrile//pentafluoropropiononitrile  
 hexafluoro-cyclopropane//Hexafluor-cyclopropan//freon-  
 20 #C216  
 Hexafluoropropylene  
 hexafluoro-[1,3]dioxolane  
 Octafluoropropane  
 Perfluormethyllethylether  
 25 1,1-difluoro-propadiene//allenylidene difluoride/1,1-dif-  
 luoro-allene  
 2,3,3,3-tetrafluoro-propene//HFO-1234yf  
 trans HFO-1234ze  
 3,3,3-Trifluoropropene  
 30 cyclopropene  
 Allene  
 1,1-difluoro-propene//propenylidene difluoride//1,1-Dif-  
 luor-propen  
 methylketene  
 35 2-fluoropropene  
 1-Propene  
 DL-2-aminopropanoic acid  
 3,3,3-trifluoro-propyne//3,3,3-Trifluor-propin//trifluorom-  
 ethyl-ethyne//3,3,3-trifluoro-1-propyne  
 40 1,1,3,3,3-pentafluoro-propene//1,1,3,3,3-Pentafluor-propen  
 1,2,3,3,3-pentafluoro-propene  
 1,1,1,4,4,4-hexafluoro-2-butyne  
 1,1,4,4-tetrafluoro-butane-2,3-dione  
 Trifluormethylhypochlorit  
 45 Chlor-difluor-methyl-hypofluorit  
 N-Chlor-N-fluor-trifluormethylamin (germ.)  
 Chlordifluordifluoraminomethan  
 thiocarbonyl difluoride  
 Thiocarbonyldifluorid (germ.)  
 50 selenocarbonyl difluoride  
 Trifluoriodomethane  
 N-Fluor-difluormethanimin (germ.)  
 trifluoro-nitroso-methane//Trifluor-nitroso-methan  
 difluoro-carbamoyl fluoride  
 55 trifluoro-nitro-methane//Trifluor-nitro-methan//fluoropicrin  
 Tetrafluoromethane  
 Tetrafluorformamidin (germ.)  
 tetrafluorourea  
 hypofluorous acid trifluoromethyl ester//Hypofluorigsaeure-  
 60 trifluormethylester//trifluoromethyl hypofluorite  
 trifluoromethanesulfonyl fluoride  
 N,N-Difluor-trifluormethylamin (germ.)  
 Trifluormethyloxydifluoramin  
 (Difluoraminoxy) difluormethylhypofluorit  
 65 sulfurcyanide pentafluoride  
 Schwefelcyanid-pentafluorid (germ.)  
 difluoro-trifluoromethyl-phosphine

Hexafluormethandiamin  
 perfluoro methyl silane  
 Perfluormethylsilan (germ.)  
 Trifluormethyl-tetrafluorphosphoran (germ.)  
 Difluoromethane  
 Fluoroiodomethane  
 fluoromethane//methyl fluoride//Fluor-methan//freon-41  
 trifluoromethyl-silane" CF<sub>3</sub>SiH<sub>3</sub>  
 methyltrifluorosilane  
 difluoro-methyl-silane  
 fluoro-methyl-silane  
 methylgermane  
 Difluorformimin  
 Trifluoromethane  
 trifluoromethane thiol  
 Trifluormethanthiol (germ.)  
 N,N,1,1-Tetrafluormethylamin  
 difluoro dichlorosilane  
 Difluordichlorsilan (germ.)  
 difluoro chlorosilane  
 Difluorchlorsilan (germ.)  
 Phosphorus chloride difluoride  
 Chlorotrifluorosilane  
 Hydrogen chloride  
 Chlorosilane  
 Carbon monoxide  
 Carbon dioxide  
 Carbonyl sulfide  
 Difluoramine  
 trans-Difluorodiazine  
 cis-Difluorodiazine  
 Thionyl fluoride  
 Trifluorosilane  
 Nitrogen trifluoride  
 Trifluoramime oxide  
 thiaetyl trifluoride  
 Phosphorus trifluoride  
 Germanium(IV) fluoride  
 Tetrafuorosilane  
 Phosphorus pentafluoride  
 Selenium hexafluoride  
 Tellurium hexafluoride  
 fluorosilane  
 Nitrosyl fluoride  
 Fluorine nitrate  
 Hydrogen sulfide  
 Ammonia  
 Helium  
 Hydrogen iodide  
 Krypton  
 Nitrogen  
 dinitrogen oxide  
 Neon  
 Nitrogen oxide; and  
 Xenon

More preferably, the dielectric compounds can be selected from the group consisting of:

Argon  
 Trifluoroborane  
 Hydrogen bromide  
 Bromopentafluoroethane  
 Chlorotrifluoroethene  
 Trifluoroacetonitrile  
 trifluoromethyl isocyanate  
 trifluoromethyl thiocarbonyl fluoride  
 Trifluormethylthiocarbonylfuorid (germ.)  
 pentafluoro-nitroso-ethane//Pentafluor-nitroso-aethan

(trifluoromethyl-carbonyl)-difluoro-amine  
 Hexafluoroethane  
 Bis-trifluormethyl-nitroxid  
 bis-trifluoromethyl ether  
 5 bis(trifluoromethyl)tellurium  
 bis(trifluoromethyl)ditelluride  
 N,N-Difluor-pentafluoraethylamin (germ.)  
 N-Fluor-bis(trifluoromethyl)-amin (germ.)  
 N-Fluor-N-trifluormethoxy-perfluormethylamin (germ.)  
 10 fluoroformyl cyanide  
 1-chloro-1-fluoro-ethene//1-Chlor-1-fluor-aethen//1-chloro-1-fluoroethylene 1,1-Difluoroethene  
 #trans!-1,2-difluoro-ethene//#trans!-vinylene difluoride//  
 15 #trans!-vinylene fluoride  
 1,2-difluoro-ethene//#cis!-vinylene difluoride//1,2-Difluor-aethen//vinylene fluoride  
 #cis!-1,2-difluoro-ethene//#cis!-vinylene difluoride//(Z)-1,2-difluoroethylene//(Z)-1,2-difluoro-ethene//#cis!-vi-  
 20 nylene fluoride  
 1,1,1,2-Tetrafluoroethane  
 1,1,2,2-Tetrafluoroethane  
 Fluoroethene  
 1,1,1-Trifluoroethane  
 25 Ether, methyl trifluoromethyl  
 Ethene  
 1,1-Difluoroethane  
 Fluoroethane  
 Ethane  
 30 fluoro-dimethyl-borane  
 Disiloxane, 1,1,3,3-tetrafluoro-1,3-dimethyl-Trifluoroethene  
 trifluoroacetaldehyde//Trifluor-acetaldehyd  
 Pentafluoroethane  
 Difluoromethyl trifluoromethyl ether  
 35 Tris(trifluoromethyl)bismuth  
 tetrafluoropropadiene//tetrafluoro-allene//1,1,3,3-tet-  
 rafuoro-1,2-propadiene  
 tetrafluorocyclopropene  
 Perfluoropropionylidod  
 40 pentafluoro-propionitrile//pentafluoropropiononitrile  
 hexafluoro-cyclopropane//Hexafluor-cyclopropan//freon-#C1216  
 Hexafluoropropylene  
 hexafluoro-[1,3]dioxolane  
 45 Octafluoropropane  
 Perfluormethyllethylether  
 1,1-difluoro-propadiene//allenylidene difluoride//1,1-difluoro-allene  
 2,3,3,3-tetrafluoro-propene//HFO-1234yf  
 50 trans HFO-1234ze  
 3,3,3-Trifluoropropene  
 cyclopropene  
 Allene  
 1,1-difluoro-propene//propenylidene difluoride//1,1-Dif-  
 55 luor-propen  
 methylketene  
 2-fluoropropene  
 1-Propene  
 DL-2-aminopropanoic acid  
 60 3,3,3-trifluoro-propyne//3,3,3-Trifluor-propin//trifluorom-ethyl-ethyne//3,3,3-trifluoro-1-propyne  
 1,1,3,3,3-pentafluoro-propene//1,1,3,3,3-Pentafluor-propen  
 1,2,3,3,3-pentafluoro-propene  
 1,1,1,4,4,4-hexafluoro-2-butyne  
 65 1,1,4,4-tetrafluoro-butane-2,3-dione  
 Trifluormethylhypochlorit  
 Chlor-difluor-methyl-hypofluorit

N-Chlor-N-fluor-trifluormethylamin (germ.)  
 Chlordifluordifluoraminomethan  
 thiocarbonyl difluoride  
 Thiocarbonyldifluorid (germ.)  
 selenocarbonyl difluoride  
 Trifluoroiodomethane  
 N-Fluor-difluormethanimin (germ.)  
 trifluoro-nitroso-methane//Trifluor-nitroso-methan  
 difluoro-carbamoyl fluoride  
 trifluoro-nitro-methane//Trifluor-nitro-methan//fluoropicrin  
 Tetrafluromethane  
 Tetrafluorformamidin (germ.)  
 tetrafluorourea  
 hypofluorous acid trifluoromethyl ester//Hypofluorigsaeure-  
 trifluormethylester//trifluoromethyl hypofluorite  
 trifluoromethanesulfonyl fluoride  
 N,N-Difluor-trifluormethylamin (germ.)  
 Trifluormethyloxydifluoramin  
 (Difluoraminoxy) difluormethylhypofluorit  
 sulfurcyanide pentafluoride  
 Schweißcyanid-pentafluorid (germ.)  
 difluoro-trifluoromethyl-phosphine  
 Hexafluormethandiamin  
 perfluoro methyl silane  
 Perfluormethylsilan (germ.)  
 Trifluoromethyl-tetrafluorphosphoran (germ.)  
 Difluoromethane  
 Fluoroiodomethane  
 fluoromethane//methyl fluoride//Fluor-methan//freon-41  
 trifluoromethyl-silane" CF<sub>3</sub>SiH<sub>3</sub>  
 methyltrifluorosilane  
 difluoro-methyl-silane  
 fluoro-methyl-silane  
 methylgermane  
 Difluorformimin  
 Trifluoromethane  
 trifluoromethane thiol  
 Trifluormethanthiol (germ.)  
 N,N,1,1-Tetrafluormethylamin  
 difluoro dichlorosilane  
 Difluordichlorsilan (germ.)  
 difluoro chlorosilane  
 Difluorchlorsilan (germ.)  
 Phosphorus chloride difluoride  
 Chlorotrifluorosilane  
 Hydrogen chloride  
 Chlorosilane  
 Carbon monoxide  
 Carbon dioxide  
 Carbonyl sulfide  
 Difluoramine  
 trans-Difluorodiazine  
 cis-Difluorodiazine  
 Thionyl fluoride  
 Trifluorosilane  
 Nitrogen trifluoride  
 Trifluoramine oxide  
 thiazyl trifluoride  
 Phosphorus trifluoride  
 Germanium(IV) fluoride  
 Tetrafuorosilane  
 Phosphorus pentafluoride  
 Selenium hexafluoride  
 Tellurium hexafluoride  
 fluorosilane  
 Nitrosyl fluoride  
 Fluorine nitrate

Hydrogen sulfide  
 Ammonia  
 Helium  
 Hydrogen iodide  
 5 Krypton  
 Nitrogen  
 Nitrous oxide  
 Neon  
 Nitrogen oxide; and  
 10 Xenon  
 The dielectric gaseous compound is optionally formed as an azeotrope, which imparts many advantages in handling the mixture. Preferred mixtures for dielectric gaseous compound contain one additional gas selected from the group consisting of: nitrogen, CO<sub>2</sub> and N<sub>2</sub>O.  
 15 The present disclosure also includes an insulation-gas for use in electrical equipment, wherein said insulation-gas is a dielectric gaseous compound which exhibits the following properties: a boiling point in the range between about -20° C.  
 20 to about -273° C.; low, preferably non-ozone depleting; a GWP less than about 22,200; chemical stability, as measured by a negative standard enthalpy of formation (dHf<0); a toxicity level such that when the dielectric gas leaks, the effective diluted concentration does not exceed its PEL (i.e., Occupational Exposure Limit (OEL or TLV) of at least about 0.3 ppm); and a dielectric strength greater than air.  
 25 Preferably, the electrical equipment is at least one selected from the group consisting of: gas-insulated circuit breakers and current-interruption equipment, gas-insulated transmission lines, gas-insulated transformers, and gas-insulated substations.

#### DETAILED DESCRIPTION OF THE PREFERRED EMBODIMENT

35 The compounds of the present disclosure are useful in gaseous phase for electrical insulation and for arc quenching and current interruption equipment used in the transmission and distribution of electrical energy. Generally, there are four  
 40 major types of electrical equipment which the gases of the present disclosure can be used for insulation and/or interruption purposes: (1) gas-insulated circuit breakers and current-interruption equipment, (2) gas-insulated transmission lines, (3) gas-insulated transformers, and (4) gas-insulated substations. Such gas-insulated equipment is a major component of power transmission and distribution systems all over the world. It offers significant savings in land use, is aesthetically acceptable, has relatively low radio and audible noise emissions, and enables substations to be installed in populated  
 45 areas close to the loads.

50 Depending on the particular function of the gas-insulated equipment, the gas properties which are the most significant vary.

55 For circuit breakers the excellent thermal conductivity and high dielectric strength of such gases, along with the fast thermal and dielectric recovery (short time constant for increase in resistivity), are the main reasons for its high interruption capability. These properties enable the gas to make a rapid transition between the conducting (arc plasma) and the dielectric state of the arc, and to withstand the rise of the recovery voltage.

60 For gas-insulated transformers the cooling ability, compatibility with solid materials, and partial discharge characteristics, added to the dielectric characteristics, make them a desirable medium for use in this type of electrical equipment. The compounds have distinct advantages over oil insulation, including none of the fire safety problems or environmental

## 11

problems related to oil, high reliability, flexible layout, little maintenance, long service life, lower noise, better handling, and lighter equipment.

For gas-insulated transmission lines the dielectric strength of the gaseous medium under industrial conditions is of paramount importance, especially the behavior of the gaseous dielectric under metallic particle contamination, switching and lightning impulses, and fast transient electrical stresses. These gases also have a high efficiency for transfer of heat from the conductor to the enclosure and are stable for long periods of time (e.g., 40 years). These gas-insulated transmission lines offer distinct advantages: cost effectiveness, high-carrying capacity, low losses, availability at all voltage ratings, no fire risk, reliability, and a compact alternative to overhead high voltage transmission lines in congested areas that avoids public concerns with overhead transmission lines.

For gas-insulated substations, the entire substation (circuit breakers, disconnects, grounding switches, busbar, transformers, etc., are interconnected) is insulated with the gaseous dielectric medium of the present disclosure, and, thus, all of the above-mentioned properties of the dielectric gas are significant.

The properties of a dielectric gas that are necessary for its use in high voltage equipment are many and vary depending on the particular application of the gas and the equipment.

Intrinsic properties are those properties of a gas which are inherent in the physical atomic or molecular structure of the gas. These properties are independent of the application or the environment in which a gas is placed. One of the desirable properties of a gaseous dielectric is high dielectric strength (higher, for instance than air). The gas properties that are principally responsible for high dielectric strength are those that reduce the number of electrons which are present in an electrically-stressed dielectric gas. To effect such a reduction in the electron number densities, as gas should: (i) be electronegative (remove electrons by attachment over as wide an energy range as possible); it should preferably exhibit increased electron attachment with increasing electron energy and gas temperature since electrons have a broad range of energies and the gas temperature in many applications is higher than ambient; (ii) have good electron slowing-down properties (slow electrons down so that they can be captured efficiently at lower energies and be prevented from generating more electrons by electron impact ionization); and (iii) have low ionization cross section and high ionization onset (prevent ionization by electron impact). Besides the above properties, there are a number of other basic properties which are necessary for the complete characterization of the dielectric gas behavior and its performance in practice, e.g., secondary processes such as electron emission from surfaces by ion and photon impact; photoprocesses; absorption of photoionizing radiation (this is a controlling factor in discharge development in non-uniform fields); dissociation under electron impact decomposition; ion-molecule reactions; reactions with trace impurities; and reactions with surfaces.

The dielectric gas must also have the following chemical properties: high vapor pressure; high specific heat, high thermal conductivity for gas cooling; thermal stability over long periods of time for temperatures greater than 400° K.; chemical stability and inertness with regard to conducting and insulating materials; non-flammable; toxicity acceptable for industrial exposure; and non-explosive. When used in mixtures, it must have appropriate thermodynamic properties for mixture uniformity, composition, and separation.

Extrinsic properties are those which describe how a gas may interact with its surroundings, or in response to external

## 12

influences, such as electrical breakdown and discharges. To be used in electrical applications, a dielectric gas should: (undergo no extensive decomposition; lead to no polymerization; form no carbon or other deposits; and be non-corrosive and non-reactive to metals, insulators, spacers, and seals. In addition it should have: no byproduct with toxicity unacceptable for industrial applications; removable byproducts; and a high recombination rate for reforming itself, especially for arc interruption. Finally, the gas must be environmentally friendly, e.g., it must not contribute to global warming, must not deplete stratospheric ozone, and must not persist in the environment for long periods of time.

Specific properties of the gas under discharge and breakdown conditions include: a high breakdown voltage under uniform and non-uniform electric fields; insensitivity to surface roughness or defects and freely moving conducting particles; good insulation properties under practical conditions; good insulator flashover characteristics; good heat transfer characteristics; good recovery (rate of voltage recovery) and self-healing; no adverse reactions with moisture and common impurities; and no adverse effects on equipment, especially on spacers and electrode surfaces.

Specific properties of gaseous insulators for specific electrical equipment is set forth below:

**Circuit breakers**—The most significant required gas properties for arc interruption are: (i) high dielectric strength comparable to that of SF<sub>6</sub>; (ii) high thermal conductivity; (iii) fast gas recovery; and (iv) self-healing/dielectric integrity.

**Gas-insulated transmission lines**—The required properties include: (i) high dielectric strength; (ii) high vapor pressure at operating and ambient temperature; (iii) chemical inertness; (iv) high thermal conductivity; (v) no thermal aging; (vi) no deposits; (vii) easily removable, non-harmful byproducts; and (viii) no unacceptable level of hazards (fire, explosion, toxicity, corrosion).

**Gas-insulated transformers**—The properties of the gas required for this application include: (i) high dielectric strength at reasonable pressures (e.g., 500 kPa); (ii) low boiling point; (iii) acceptably low toxicity; (iv) chemical inertness; (v) good thermal stability; (vi) non-flammable; (vii) high cooling capability; (viii) good compatibility with solid materials; (ix) good partial discharge characteristics; (x) useable over a range of temperatures; and (xi) safe, easy to handle, inexpensive and securely available.

The present inventors have discovered a unique series of dielectric gases for use in electric equipment applications, which exhibit many of the aforementioned properties, which avoiding the greenhouse problems associated with SF<sub>6</sub>. Such dielectric compounds exhibit at least one of the following properties:

A boiling point in the range between about -20° C. to about -273° C.

Low, preferably, Non-ozone depleting  
A GWP less than about 22,200

Chemical stability, as measured by a negative standard enthalpy of formation (dHf<0)

A toxicity level such that when the working gas leaks from equipment at the manufacturer's specified maximum leak rate, the effective diluted concentration does not exceed its PEL, i.e., does not exceed the PEL of that specific compound. In general with minimal ventilation PELs greater than about 0.3 ppm by volume are acceptable (i.e., an Occupational Exposure Limit (OEL or

TLV) of at least about 0.3 ppm). OSHA sets enforceable permissible exposure limits (PELs) to protect workers against the health effects of exposure to hazardous substances. OSHA PELs are based on an 8-hour time weighted average (TWA) exposure. Approximately 500 PELs have been established. Existing PELs are con-

tained in 29 CFR 1910.1000, the air contaminants standard. Most PELs are listed in 29 CFR 1910.1000, Table Z-1, and 29 CFR 1910.1000, Table Z-2.

A dielectric strength greater than air.

5 These unique dielectric gases are at least one gas selected from the group consisting of those set forth in Table 1 below:

TABLE 1

| Dielectric Compound | Structure                      | Name                                                           | CAS        | MW     | MY BP(° C.) |
|---------------------|--------------------------------|----------------------------------------------------------------|------------|--------|-------------|
| AsF5                | AsF5                           | Arsenic pentafluoride                                          | 7784-36-3  | 169.91 | -52.8       |
| AsH3                | AsH3                           | Arsine                                                         | 7784-42-1  | 77.95  | -62.2       |
| B2F4                | B2F4                           | Diboron tetrafluoride                                          | 13965-73-6 | 97.61  | -34.2       |
| B2H6                | H2B(H2)BH2                     | Diborane                                                       | 19287-45-7 | 27.67  | -92.3       |
| C2Cl2F4O4           | O3ClOCF2CF2Cl                  | Perchloric acid, 2-chloro-1,1,2,2-tetrafluoroethyl ester (9Cl) | 38126-28-2 | 234.92 | -95.0       |
| C2Cl4F2O4           | O3ClOCFC1CFC12                 | Perchloric acid, 1,2,2-trichloro-1,2-difluoroethyl ester       | 38126-29-3 | 267.83 | -35.0       |
| C2ClF3O             | CF3CCl(O)                      | Trifluoroacetyl chloride                                       | 354-32-5   | 132.47 | -27.0       |
| C2F3N               | (CF3)---NC                     | trifluoromethylisocyanide (CF3---NC)                           | 19480-01-4 | 95.02  | -84.0       |
| C2F3N               | CF3---NC                       | trifluoromethyl isocyanide                                     | 19480-01-4 | 95.02  | -35.0       |
| C2F3NO              | CF2=CF---NO                    | trifluoro-nitroso-ethene//Trifluor-nitroso-<br>aethen          | 2713-04-4  | 111.02 | -23.7       |
| C2F4                | C2F4                           | Tetrafluoroethene                                              | 116-14-3   | 100.02 | -75.6       |
| C2F4N2              | cyclo---CF2---N---N---CF2---   | 3,3,4,4-tetrafluoro-3,4-dihydro-[1,2]diazete                   | 694-60-0   | 128.03 | -36.0       |
| C2F4N2              | NF2---CF2---CN                 | (Difluoramino)difluoracetonitril                               | 5131-88-4  | 128.03 | -32.0       |
| C2F4O               | O(CF2CF2)                      | Tetrafluorooxirane                                             | 694-17-7   | 116.01 | -63.5       |
| C2F4O               | CF3CF(O)                       | Trifluoroacetyl fluoride                                       | 354-34-7   | 116.01 | -59.0       |
| C2F4O2              | FC(O)OCF3                      | Perfluoromethylfluorformiat                                    | 3299-24-9  | 132.01 | -33.0       |
| C2F4O2              | CF3C(O)OF                      | trifluoro-acetyl hypofluorite                                  | 359-46-6   | 132.01 | -25.0       |
| C2F5N               | CF3N=CF2                       | perfluoro-2-aza-1-propene                                      | 133.02     | 133.02 | -34.0       |
| C2F5N               | CF3CFNF                        | Perfluor-2-aza-1-propen (germ.)                                | 758-35-0   | 133.02 | -32.0       |
| C2F5NO              | cyclo---CF2---N(CF3)---O---    | N-Fluor-tetrafluor-1-aethanimin (germ.)                        | 60247-20-3 | 149.02 | -34.8       |
| C2F6N2              | (CF3)N=N(CF3)                  | 3,3-difluoro-2-trifluoromethyl-oxaziridine                     | 372-63-4   | 166.03 | -20.0       |
| C2F6O               | C2F5OF                         | bis-trifluoromethyl-diazene//hexafluoro-#cis!-azomethane       | 3848-94-0  | 154.01 | -50.0       |
| C2F6O2              | CF3---O---O---CF3              | Fluoroxypentafluoroethane                                      | 927-84-4   | 170.01 | -40.0       |
| C2F6O2              | CF3C(OF)2F                     | bis-trifluoromethyl peroxide                                   | 16329-92-3 | 170.01 | -35.0       |
| C2F6S               | (CF3)2S                        | Bis(fluoroxy)tetrafluoroethan                                  | 371-78-8   | 170.08 | -22.2       |
| C2FN3               | (---N---N---)                  | Hexafluorodimethyl sulfide                                     | 4849-85-8  | 85.04  | -30.0       |
|                     | CF(CN)                         | 3-fluoro-3#H!-diazirine-3-carbonitrile                         |            |        |             |
| C2H2                | HCCH                           | Ethyne                                                         | 74-86-2    | 26.04  | -84.7       |
| C2H2F3N             | ---CF2---NF---CH2---           | 1,2,2-trifluoro-aziridine                                      | 1514-44-9  | 97.04  | -24.0       |
| C2H2O               | CH2CO                          | Ketene                                                         | 463-51-4   | 42.04  | -49.8       |
| C2H3BF2             | F2BCHCH2                       | (difluoro)vinyllboran                                          | 358-95-2   | 75.85  | -38.8       |
| C2H3FSi             | F3Si---CH=CH2                  | (Difluor)vinyllboran (germ.)                                   | 421-24-9   | 112.13 | -25.0       |
| C2H4Si              | HCCSiH3                        | trifluoro-vinyl-silane                                         | 1066-27-9  | 56.14  | -22.4       |
| C2H5BF2             | (C2H5)F2B                      | Ethinyllsilan                                                  | 430-41-1   | 77.87  | -25.0       |
| C2H5N               | CH2=NCH3                       | Ethyl-difluor-boran (germ.)                                    |            |        |             |
| C2H6O               | CH3OCH3                        | methyl-methylen-amine                                          | 1761-67-7  | 43.07  | -35.0       |
| C2H6Si              | H2CCSiH3                       | Dimethyl ether                                                 | 115-10-6   | 46.07  | -24.8       |
| C2H8Si              | (CH3)2SiH2                     | vinyl-silane                                                   | 7291-09-0  | 58.15  | -22.8       |
| C2HCl               | C1CCH                          | Dimethylsilane                                                 | 1111-74-6  | 60.17  | -20.2       |
| C2HF                |                                | Chloroethyne                                                   | 593-63-5   | 60.48  | -30.2       |
|                     |                                | fluoroethyne//fluoro-acetylene                                 | 2713-09-9  | 44.03  | -105.0      |
| C2N2                | NCCN                           | Ethanedinitrile                                                | 460-19-5   | 52.03  | -21.2       |
| C3F4                | FCCCC3                         | tetrafluoropropyne//1,3,3,3-tetrafluoropropyne                 | 20174-11-2 | 112.03 | -50.0       |
| C3F6O               | cyclo---CF2---CF2---O---CF2--- | hexafluoro-oxetane                                             | 425-82-1   | 166.02 | -38.0       |
| C3F6O               | cyclo---CF2---O---CF(CF3)---   | Trifluoro(trifluoromethyl)oxirane                              | 428-59-1   | 166.02 | -27.4       |
| C3F6O               | (CF3)2CO                       | 1,1,1,3,3,3-Hexafluoropropanone                                | 684-16-2   | 166.02 | -27.3       |

TABLE 1-continued

| Dielectric Compound | Structure           | Name                                                         | CAS        | MW     | MY BP(° C.) |
|---------------------|---------------------|--------------------------------------------------------------|------------|--------|-------------|
| C3F6O               | CF3CF2C(O)F         | pentafluoro-propionyl fluoride//perfluoropropionyl fluoride  | 422-61-7   | 166.02 | -27.0       |
| C3F6O               | CF3OCFCF2           | Trifluoromethyl trifluorovinyl ether                         | 1187-93-5  | 166.02 | -26.0       |
| C3H4                | CH3CCH              | 1-Propyne                                                    | 74-99-7    | 40.06  | -23.2       |
| C3H6                | —CH2CH2CH2—         | Cyclopropane                                                 | 75-19-4    | 42.08  | -32.8       |
| C3H8                | CH3CH2CH3           | Propane                                                      | 74-98-6    | 44.10  | -42.0       |
| C3H9B               | B(CH3)3             | Trimethylborane                                              | 593-90-8   | 55.92  | -20.2       |
| C3HNO               | OCCHCN              | cyanoketene                                                  | 4452-08-8  | 67.05  | -34.0       |
| C4H4                | CH2=C=C=CH2         | butatriene                                                   | 2873-50-9  | 52.08  | -78.0       |
| C5F10NP             | (C2F5)2PCN          | Cyano-bis(pentafluoroethyl)-phosphin                         | 35449-90-2 | 295.02 | -78.0       |
| C5H10F4Si           | CHF2CF2Si(CH3)3     | Trimethyl-1,1,2,2-tetrafluoroethylsilan                      | 4168-08-5  | 174.21 | -72.0       |
| CB2H8               | CH3B2H5             | methyl diborane                                              | 23777-55-1 | 41.70  | -35.0       |
| CBrFO               | COBrF               | Methyldiboran (germ.)                                        | 753-56-0   | 126.91 | -20.6       |
| CClF2NO             | (F2Cl)CN=O          | carbonyl bromide fluoride                                    | 421-13-6   | 115.47 | -35.0       |
| CClF3O2             | CF3—O—O—Cl          | chloroperoxytrifluoromethane                                 | 32755-26-3 | 136.46 | -22.0       |
| CClFO               | COClF               | carbonylchlorid-fluorid                                      | 353-49-1   | 82.46  | -46.0       |
| CF2N2               | F2C(—N=N—)          | Carbonychloridfluorid (germ.)                                |            |        |             |
| CF2N2               | F2C=N=N             | 3,3-difluoro-3#H1-diazirine                                  | 693-85-6   | 78.02  | -91.3       |
|                     |                     | difluoro diazomethane                                        | 814-73-3   | 78.02  | -91.3       |
|                     |                     | Difluordiazomethan (germ.)                                   |            |        |             |
| CF2O                | F2CO                | Carbonyl fluoride                                            | 353-50-4   | 66.01  | -84.6       |
| CF2O2               | F2C(OO)             | Difluordioxiran                                              | 96740-99-7 | 82.01  | -85.0       |
| CF3N3               | (NF2)(F)C(—N=N—)    | difluoro-(3-fluoro-3#H1-diazirin-3-yl)-amine                 | 4823-43-2  | 111.03 | -36.0       |
| CF3N3               | CF3—N—N—N           | trifluoromethylazide                                         | 3802-95-7  | 110.03 | -28.5       |
| CF4N2               | cyclo-(—NF—NF—CF2—) | Trifluormethylazid (germ.)                                   |            |        |             |
| CF4O2               | CF3—O—O—F           | tetrafluoro-diaziridine                                      | 17224-09-8 | 116.02 | -35.0       |
| CF4O2               | F2C(OF)2            | Fluorperoxytrifluoromethan                                   | 34511-13-2 | 120.00 | -69.4       |
| CF5OP               | OPF2CF3             | Bis(fluoroxy)difluormethan                                   | 16282-67-0 | 120.00 | -64.0       |
| CFN                 |                     | Trifluormethyl-phosphonylfluorid                             | 19162-94-8 | 153.98 | -20.1       |
| CH2F3P              | CF3PH2              | Cyanogen fluoride                                            | 1495-50-7  | 45.02  | -46.2       |
|                     |                     | Trifluoromethylphosphane (germ.)                             | 420-52-0   | 102.00 | -26.5       |
| CH2N2               | H2CNN               | Diazomethane                                                 | 334-88-3   | 42.04  | -23.2       |
| CH2O                |                     | formaldehyde//Formalin                                       | 50-00-0    | 30.03  | -21.0       |
| CH3BF2              | CH3BF2              | (methyl)difluoroborane                                       | 373-64-8   | 63.84  | -62.3       |
|                     |                     | (Methyl)difluoroborane (germ.)                               |            |        |             |
| CH3Cl               | CH3Cl               | Chloromethane                                                | 74-87-3    | 50.49  | -24.2       |
| CH3F2P              | F2PCH3              | methylphosphorous acid difluoride//difluoro-methyl-phosphine | 84.01      | -28.0  |             |
| CH3F3OSi            | F3Si—O—CH3          | trifluoro-methoxy-silane                                     | 25711-11-9 | 116.11 | -78.0       |
| CH3FO               | CH3—O—F             | Methylhypofluorid                                            | 36336-08-0 | 50.03  | -33.0       |
| CH4                 | CH4                 | Methane                                                      | 74-82-8    | 16.04  | -161.5      |
| CH6Si               | CH3SiH3             | Methylsilane                                                 | 992-94-9   | 46.14  | -56.9       |
| CH7BrSi2            | H3Si—CH2—SiH2Br     | #Si!-bromo-#Si!,#Si!'-methanediyl-bis-silane                 | 56962-86-8 | 155.14 | -64.0       |
| CH7Si2              | H3Si—CH2—SiH2I      | #Si!-iodo-#Si!,#Si!'-methanediyl-bis-silane                  | 56962-87-9 | 202.14 | -49.0       |
| CHF2NO2             | F2CH—O—NO           | Difluomethylnitrit                                           | 1493-06-7  | 97.02  | -20.0       |
| CHF3O               | F3COH               | trifluoromethanol                                            | 1493-11-4  | 86.01  | -20.0       |
| CHFO                | HFCO                | Formyl fluoride                                              | 1493-02-3  | 48.02  | -26.5       |
| CHNO                | HOCH                | Cyanic acid                                                  | 420-05-3   | 43.03  | -64.2       |
| Cl2                 | Cl2                 | Chlorine                                                     | 7782-50-5  | 70.91  | -34.0       |
| CIF                 | CIF                 | Chlorine fluoride                                            | 7790-89-8  | 54.45  | -101.0      |
| ClFO3               |                     | Chlorine trioxide fluoride                                   | 7616-94-6  | 102.45 | -46.7       |
| COSe                | Se=C=O              | carbon oxide                                                 | 1603-84-5  | 106.97 | -21.7       |
|                     |                     | selenide//Kohlenoxidseleinid                                 |            |        |             |
| F2                  | F2                  | Fluorine                                                     | 7782-41-4  | 38.00  | -188.2      |
| F2H2Si              | SiF2H2              | Difluorosilane                                               | 13824-36-7 | 68.10  | -77.8       |
| F2O                 | OF2                 | Fluorine oxide                                               | 7783-41-7  | 54.00  | -144.7      |
| F2O2                | FOOF                | fluorine peroxide                                            | 7783-44-0  | 70.00  | -57.0       |
| F2O2S               | SO2F2               | Sulfuryl fluoride                                            | 2699-79-8  | 102.06 | -55.3       |
| F2S                 | SF2                 | sulphur difluoride                                           | 13814-25-0 | 70.06  | -35.0       |
| F3OP                | POF3                | Phosphorus trifluoride oxide                                 | 13478-20-1 | 103.97 | -39.7       |

TABLE 1-continued

| Dielectric Compound | Structure  | Name                                                                                                                                  | CAS        | MW     | MY BP(° C.) |
|---------------------|------------|---------------------------------------------------------------------------------------------------------------------------------------|------------|--------|-------------|
| F3PS                | PSF3       | Phosphorus trifluoride sulfide                                                                                                        | 2404-52-6  | 120.03 | -52.3       |
| F4HP                | PHF4       | tetrafluorophosphorane                                                                                                                | 13659-66-0 | 107.98 | -37.0       |
| F4N2                | F2NNF2     | Tetrafluorohydrazine                                                                                                                  | 10036-47-2 | 104.01 | -74.2       |
| F4S                 | SF4        | Sulfur tetrafluoride                                                                                                                  | 7783-60-0  | 108.05 | -40.5       |
| F6OSi2              | SiF3OSiF3  | hexafluoro disiloxane                                                                                                                 | 14515-39-0 | 186.16 | -23.0       |
|                     |            | Hexafluorodisiloxan (germ.)                                                                                                           |            |        |             |
| FNO2                | O2NF       | Nitryl fluoride                                                                                                                       | 10022-50-1 | 65.00  | -72.3       |
| H2                  | H2         | Hydrogen                                                                                                                              | 1333-74-0  | 2.02   | -252.9      |
| H2Se                | H2Se       | Hydrogen selenide                                                                                                                     | 7783-07-5  | 80.98  | -41.3       |
| H3P                 | PH3        | Phosphorus trihydride                                                                                                                 | 7803-51-2  | 34.00  | -87.8       |
| H4Ge                | GeH4       | Germanium hydride                                                                                                                     | 7782-65-2  | 76.62  | -88.2       |
| H4Si                | SiH4       | Silane                                                                                                                                | 7803-62-5  | 32.12  | -112.2      |
| H4Sn                | SnH4       | Tin tetrahydride                                                                                                                      | 2406-52-2  | 122.72 | -51.8       |
| O2                  | O2         | Oxygen                                                                                                                                | 7782-44-7  | 32.00  | -183.0      |
| O3                  | O3         | Ozone                                                                                                                                 | 10028-15-6 | 48.00  | -111.3      |
| PSb                 | SbP        | Antimony monophosphide                                                                                                                | na         | 152.72 | -52.3       |
| PSi2                | Si2P       | Disilicon monophosphide                                                                                                               | na         | 87.14  | -52.3       |
| Rn                  | Rn         | Radon                                                                                                                                 | 10043-92-2 | 222.00 | -61.7       |
| Ar                  | Ar         | Argon                                                                                                                                 | 7440-37-1  | 39.95  | -185.9      |
| BF3                 | BF3        | Trifluoroborane                                                                                                                       | 7637-07-2  | 67.81  | -101.2      |
| BrH                 | HBr        | Hydrogen bromide                                                                                                                      | 10035-10-6 | 80.91  | -66.7       |
| C2BrF5              | CF3CF2Br   | Bromopentafluoroethane                                                                                                                | 354-55-2   | 198.92 | -21.0       |
| C2ClF3              | CFCl=CF2   | Chlorotrifluoroethene                                                                                                                 | 79-38-9    | 116.47 | -28.4       |
| C2F3N               | CF3CN      | Trifluoroacetonitrile                                                                                                                 | 353-85-5   | 95.02  | -68.8       |
| C2F3NO              | (CF3)NCO   | trifluoromethyl isocyanate                                                                                                            | 460-49-1   | 111.02 | -36.0       |
| C2F4S               | CF3C(S)F   | trifluoromethyl thiocarbonyl fluoride                                                                                                 |            | 132.08 | -21.0       |
|                     |            | Trifluoromethylthiocarbonylfluorid (germ.)                                                                                            |            |        |             |
| C2F5NO              | CF3CF2NO   | pentafluoro-nitroso-ethane//Pentafluor-nitroso-aethan                                                                                 | 354-72-3   | 149.02 | -45.7       |
| C2F5NO              | CF3C(O)NF2 | (trifluoromethyl-carbonyl)-difluoro-amine                                                                                             | 32822-49-4 | 149.02 | -21.1       |
| C2F6                | CF3CF3     | Hexafluoroethane                                                                                                                      | 76-16-4    | 138.01 | -78.2       |
| C2F6NO              | CF3N(O)CF3 | Bis-trifluoromethyl-nitroxid                                                                                                          | 2154-71-4  | 168.02 | -20.0       |
| C2F6O               | CF3OCF3    | bis-trifluoromethyl ether                                                                                                             | 1479-49-8  | 154.01 | -59.0       |
| C2F6Te              | (CF3)2Te   | bis(trifluoromethyl)tellurium                                                                                                         | 55642-42-7 | 265.61 | -98.0       |
| C2F6Te2             | CF3TeCF3   | bis(trifluoromethyl)ditelluride                                                                                                       | 1718-20-3  | 393.21 | -53.0       |
| C2F7N               | CF3CF2NF2  | N,N-Difluor-pentafluoroethylamin (germ.)                                                                                              | 354-80-3   | 171.02 | -38.0       |
| C2F7N               | (CF3)2NF   | N-Fluor-bis(trifluoromethyl)-amin (germ.)                                                                                             | 359-62-6   | 171.02 | -37.0       |
| C2F7NO              | CF3NFOCF3  | N-Fluor-N-trifluormethoxy-perfluoromethylamin (germ.)                                                                                 | 4217-92-9  | 187.02 | -25.0       |
| C2FNO               | FC(O)CN    | fluoriformyl cyanide                                                                                                                  | 683-55-6   | 73.03  | -21.0       |
| C2H2ClF             | CH2CFC1    | 1-chloro-1-fluoro-ethene//1-Chlor-1-fluor-aethen//1-chloro-1-fluoroethylene                                                           | 2317-91-1  | 80.49  | -25.5       |
| C2H2F2              | CF2=CH2    | 1,1-Difluoroethene                                                                                                                    | 75-38-7    | 64.03  | -85.7       |
| C2H2F2              | CHF=CHF    | #trans-1,2-difluoro-ethene//#trans-1,2-difluoro-ethylene//(E)-1,2-difluoroethylene//(E)-1,2-difluoro-ethene//#trans-vinylene fluoride | 1630-78-0  | 64.03  | -53.1       |
| C2H2F2              | FHC=CHF    | 1,2-difluoro-ethene//cis-vinylene fluoride//1,2-Difluor-aethen/vinylene fluoride                                                      | 1691-13-0  | 64.03  | -28.0       |
| C2H2F2              | CHF=CHF    | #cis-1,2-difluoro-ethene//#cis-vinylene difluoride//(Z)-1,2-difluoroethylene//(Z)-1,2-difluoro-ethene//#cis-vinylene fluoride         | 1630-77-9  | 64.03  | -26.0       |
| C2H2F4              | CF3CH2F    | 1,1,1,2-Tetrafluoroethane                                                                                                             | 811-97-2   | 102.03 | -26.1       |
| C2H2F4              | CF2HCF2H   | 1,1,2,2-Tetrafluoroethane                                                                                                             | 359-35-3   | 102.03 | -23.0       |
| C2H3F               | CH2=CHF    | Fluoroethene                                                                                                                          | 75-02-5    | 46.04  | -72.2       |
| C2H3F3              | CF3CH3     | 1,1,1-Trifluoroethane                                                                                                                 | 420-46-2   | 84.04  | -47.3       |
| C2H3F3O             | F3COCH3    | Ether, methyl trifluoromethyl                                                                                                         | 421-14-7   | 100.04 | -24.0       |
| C2H4                | H2CCH2     | Ethene                                                                                                                                | 74-85-1    | 28.05  | -103.7      |
| C2H4F2              | CHF2CH3    | 1,1-Difluoroethane                                                                                                                    | 75-37-6    | 66.05  | -24.0       |
| C2H5F               | CH3CH2F    | Fluoroethane                                                                                                                          | 353-36-6   | 48.06  | -37.7       |

TABLE 1-continued

| Dielectric Compound | Structure              | Name                                                                                              | CAS         | MW     | MY BP(° C.) |
|---------------------|------------------------|---------------------------------------------------------------------------------------------------|-------------|--------|-------------|
| C2H6                | CH3CH3                 | Ethane                                                                                            | 74-84-0     | 30.07  | -88.6       |
| C2H6BF              | (CH3)2BF               | fluoro-dimethyl-borane                                                                            | 353-46-8    | 59.88  | -44.0       |
| C2H6F4OSi2          | CH3SiF2OSiF2CH3        | Disiloxane, 1,1,3,3-tetrafluoro-1,3-dimethyl-                                                     | 63089-45-2  | 178.23 | -39.0       |
| C2HF3               | CF2=CFH                | Trifluoroethene                                                                                   | 359-11-5    | 82.02  | -51.0       |
| C2HF3O              | CF3C(O)H               | trifluoroacetaldehyde//Trifluor-acetaldehyd                                                       | 75-90-1     | 98.02  | -21.0       |
| C2HF5               | CF3CF2H                | Pentafluoroethane                                                                                 | 354-33-6    | 120.02 | -48.1       |
| C2HF5O              | CF3OCHF2               | Difluoromethyl trifluoromethyl ether                                                              | 3822-68-2   | 136.02 | -35.3       |
| C3BiF9              | Bi(CF3)3               | Tris(trifluoromethyl)bismuth                                                                      | 5863-80-9   | 416.00 | -55.0       |
| C3F4                | F2C=C=CF2              | tetrafluoropropadiene//tetrafluoro-allene//1,1,3-tetrafluoro-1,2-propadiene                       | 461-68-7    | 112.03 | -38.0       |
| C3F4                | =CFCF2CF=              | tetrafluorocyclopropene                                                                           | 19721-29-0  | 112.03 | -20.0       |
| C3F5IO              | CF3CF2C(O)I            | Perfluoropropionyl iodid                                                                          | 137741-03-8 | 273.93 | -27.0       |
| C3F5N               | C2F5CN                 | pentafluoropropionitrile//pentafluoropropiononitrile                                              | 422-04-8    | 145.03 | -35.0       |
| C3F6                | cyclo-<br>—CF2CF2CF2—  | hexafluoro-cyclopropane//Hexafluor-cyclopropan//freon-#C1216                                      | 931-91-9    | 150.02 | -33.0       |
| C3F6                | CF3CF=CF2              | Hexafluoropropylene                                                                               | 116-15-4    | 150.02 | -29.6       |
| C3F6O2              | cyclo-CF2—O—CF2—CF2—O— | hexafluoro-[1,3]dioxolane                                                                         | 21297-65-4  | 182.02 | -22.1       |
| C3F8                | CF3CF2CF3              | Octafluoropropane                                                                                 | 76-19-7     | 188.02 | -36.7       |
| C3F8O               | CF3CF2OCF3             | Perfluoromethyl ethylether                                                                        | 665-16-7    | 204.02 | -20.0       |
| C3H2F2              | F2CCH2                 | 1,1-difluoro-propadiene//allenylidene difluoride//1,1-difluoro-allene                             | 430-64-8    | 76.05  | -21.0       |
| C3H2F4              | H2CCFCF3               | 2,3,3,3-tetrafluoro-propene//HFO-1234yf                                                           | 754-12-1    | 114.04 | -28.3       |
| C3H2F4              | CHF=CHCF3              | trans HFO-1234ze                                                                                  |             | 114.04 | -19.0       |
| C3H3F3              | CH2=CHCF3              | 3,3,3-Trifluoropropene                                                                            | 677-21-4    | 96.05  | -25.0       |
| C3H4                | c-(CH=CH—CH2)          | cyclopropene                                                                                      | 2781-85-3   | 40.06  | -36.0       |
| C3H4                | H2CCH2                 | Allene                                                                                            | 463-49-0    | 40.06  | -34.5       |
| C3H4F2              | CH3CH=CF2              | 1,1-difluoro-propene//propenylidene difluoride//1,1-Difluor-propen                                | 430-63-7    | 78.06  | -29.0       |
| C3H4O               |                        | methylketene                                                                                      | 6004-44-0   | 56.06  | -23.0       |
| C3H5F               | CH2CFCH3               | 2-fluoropropene                                                                                   | 1184-60-7   | 60.07  | -24.0       |
| C3H6                | CH2CHCH3               | 1-Propene                                                                                         | 115-07-1    | 42.08  | -47.7       |
| C3H7NO2             |                        | DL-2-aminopropanoic acid                                                                          | 302-72-7    | 89.09  | -50.2       |
| C3HF3               | F3CCCH                 | 3,3,3-trifluoro-propyne//3,3,3-Trifluor-propin//trifluoromethyl-ethyne//3,3,3-trifluoro-1-propyne | 661-54-1    | 94.04  | -48.0       |
| C3HF5               | CF3CH=CF2              | 1,1,3,3,3-pentafluoro-propene//1,1,3,3,3-Pentafluor-propen                                        | 690-27-7    | 132.03 | -21.0       |
| C3HF5               | CF3—CF—CFH             | 1,2,3,3,3-pentafluoro-propene                                                                     | 2252-83-7   | 132.03 | -20.0       |
| C4F6                | CF3CCCCF3              | 1,1,1,4,4,4-hexafluoro-2-butyne                                                                   | 692-50-2    | 162.03 | -24.6       |
| C4H2F4O2            | CF2HC(O)C(O)CF2H       | 1,1,4,4-tetrafluoro-butane-2,3-dione                                                              |             | 158.05 | -81.0       |
| C4H6N2O2            |                        |                                                                                                   |             | 114.10 | -33.0       |
| CCIF3O              | F3C—O—Cl               | Trifluoromethylhypochlorit                                                                        | 22082-78-6  | 120.46 | -47.0       |
| CCIF3O              | ClF2C—OF               | Chlor-difluor-methyl-hypofluorit                                                                  | 20614-17-9  | 120.46 | -25.0       |
| CCIF4N              | CF3NFC1                | N-Chlor-N-fluor-trifluoromethylamin (germ.)                                                       | 13880-72-3  | 137.46 | -32.8       |
| CCIF4N              | C1CF2—NF2              | Chlordifluorodifluoraminomethan                                                                   | 13880-71-2  | 137.46 | -28.0       |
| CF2S                | F2C=S                  | thiocarbonyl difluoride                                                                           | 420-32-6    | 82.07  | -46.0       |
|                     |                        | Thiocarbonyldifluorid (germ.)                                                                     |             |        |             |
| CF2Se               | F2C=Se                 | selenocarbonyl difluoride                                                                         | 54393-39-4  | 128.97 | -28.0       |
| CF3I                | CF3I                   | Trifluoroiodomethane                                                                              | 2314-97-8   | 195.91 | -21.8       |
| CF3N                | CF2—N—F                | N-Fluor-difluormethanimin (germ.)                                                                 | 338-66-9    | 83.01  | -101.0      |
| CF3NO               | CF3N=O                 | trifluoro-nitroso-methane//Trifluor-nitroso-methan                                                | 334-99-6    | 99.01  | -86.0       |

TABLE 1-continued

| Dielectric Compound               | Structure                                       | Name                                                                                                         | CAS        | MW     | MY BP(° C.) |
|-----------------------------------|-------------------------------------------------|--------------------------------------------------------------------------------------------------------------|------------|--------|-------------|
| CF <sub>3</sub> NO                | FC(O)NF <sub>2</sub>                            | difluoro-carbamoyl fluoride                                                                                  | 2368-32-3  | 99.01  | -52.0       |
| CF <sub>3</sub> NO <sub>2</sub>   | CF <sub>3</sub> NO <sub>2</sub>                 | trifluoro-nitro-methane//Trifluor-nitro-methan//fluoropicrin                                                 | 335-02-4   | 115.01 | -33.6       |
| CF <sub>4</sub>                   | CF <sub>4</sub>                                 | Tetrafluoromethane                                                                                           | 75-73-0    | 88.00  | -128.1      |
| CF <sub>4</sub> N <sub>2</sub>    | NF <sub>2</sub> CF=NF                           | Tetrafluorformamidin (germ.)                                                                                 | 14362-70-0 | 116.02 | -30.0       |
| CF <sub>4</sub> N <sub>2</sub> O  | (NF <sub>2</sub> ) <sub>2</sub> CO              | tetrafluorourea                                                                                              | 10256-92-5 | 132.02 | -20.0       |
| CF <sub>4</sub> O                 |                                                 | hypofluorous acid trifluoromethylester//Hypofluorigsaeure-trifluoromethylester//trifluoromethyl hypofluorite |            | 104.00 | -95.0       |
| CF <sub>4</sub> O <sub>2</sub> S  | CF <sub>3</sub> SO <sub>2</sub> F               | trifluoromethanesulfonyl fluoride                                                                            | 335-05-7   | 152.07 | -21.7       |
| CF <sub>5</sub> N                 | CF <sub>3</sub> NF <sub>2</sub>                 | N,N-Difluor-trifluormethylamin (germ.)                                                                       | 335-01-3   | 121.01 | -75.0       |
| CF <sub>5</sub> NO                | CF <sub>3</sub> ONF <sub>2</sub>                | Trifluoromethyloxidifluoramin (Difluoraminoxy)disfluoromethyl-hypofluorit                                    | 4217-93-0  | 137.01 | -59.8       |
| CF <sub>5</sub> NO <sub>2</sub>   | F <sub>2</sub> NOCF <sub>2</sub> OF             | (Difluoraminoxy)disfluoromethyl-hypofluorit                                                                  | 36781-60-9 | 153.01 | -29.0       |
| CF <sub>5</sub> NS                | SF <sub>5</sub> CN                              | sulfurcyanide pentafluoride                                                                                  | 1512-13-6  | 153.08 | -25.0       |
| CF <sub>5</sub> P                 | CF <sub>3</sub> PF <sub>2</sub>                 | Schwefelycyanid-pentafluorid (germ.)                                                                         |            |        |             |
|                                   |                                                 | difluoro-trifluoromethyl-phosphine                                                                           | 1112-04-5  | 137.98 | -43.0       |
| CF <sub>6</sub> N <sub>2</sub>    | F <sub>2</sub> NCF <sub>2</sub> NF <sub>2</sub> | Hexafluormethandiamin                                                                                        | 4394-93-8  | 154.01 | -37.0       |
| CF <sub>6</sub> Si                | CF <sub>3</sub> SiF <sub>3</sub>                | perfluoro methyl silane                                                                                      | 335-06-8   | 154.09 | -42.0       |
| CF <sub>7</sub> P                 | CF <sub>3</sub> PF <sub>4</sub>                 | Perfluormethylsilan (germ.)                                                                                  |            |        |             |
|                                   |                                                 | Trifluoromethyl-tetrafluorophosphoran (germ.)                                                                | 1184-81-2  | 175.97 | -35.0       |
| CH <sub>2</sub> F <sub>2</sub>    | CH <sub>2</sub> F <sub>2</sub>                  | Difluoromethane                                                                                              | 75-10-5    | 52.02  | -51.7       |
| CH <sub>2</sub> FI                | CH <sub>2</sub> FI                              | Fluoroiodomethane                                                                                            | 373-53-5   | 159.93 | -53.8       |
| CH <sub>3</sub> F                 |                                                 | fluoromethane/methyl fluoride//Fluormethan//freon-41                                                         | 593-53-3   | 34.03  | -78.3       |
| CH <sub>3</sub> F <sub>3</sub> Si | CF <sub>3</sub> SiH <sub>3</sub>                | trifluoromethyl-silane"                                                                                      | 10112-11-5 | 100.12 | -38.3       |
| CH <sub>3</sub> F <sub>3</sub> Si | CH <sub>3</sub> SiF <sub>3</sub>                | CF <sub>3</sub> SiH <sub>3</sub>                                                                             |            |        |             |
| CH <sub>4</sub> F <sub>2</sub> Si | F <sub>2</sub> HSiCH <sub>3</sub>               | methyltrifluorosilane                                                                                        | 373-74-0   | 100.12 | -30.0       |
| CH <sub>5</sub> FSi               | CH <sub>3</sub> SiH <sub>2</sub> F              | difluoro-methyl-silane                                                                                       | 420-34-8   | 82.12  | -35.6       |
| CH <sub>6</sub> Ge                | H <sub>3</sub> GeCH <sub>3</sub>                | fluoro-methyl-silane                                                                                         | 753-44-6   | 64.13  | -44.0       |
| CH <sub>7</sub> F <sub>2</sub> N  | F <sub>2</sub> C=N                              | methylgermane                                                                                                | 1449-65-6  | 90.65  | -23.0       |
| CH <sub>7</sub> F <sub>3</sub>    | CHF <sub>3</sub>                                | Difluorformimin                                                                                              | 2712-98-3  | 65.02  | -22.0       |
| CH <sub>7</sub> F <sub>3</sub> S  | CF <sub>3</sub> SH                              | Trifluoromethane                                                                                             | 75-46-7    | 70.01  | -82.1       |
|                                   |                                                 | trifluoromethane thiol                                                                                       | 1493-15-8  | 102.08 | -36.7       |
| CH <sub>7</sub> F <sub>4</sub> N  | CF <sub>2</sub> H—NF <sub>2</sub>               | Trifluoromethan thiol (germ.)                                                                                |            |        |             |
|                                   |                                                 | N,N,1,1-                                                                                                     | 24708-53-0 | 103.02 | -43.0       |
| Cl <sub>2</sub> F <sub>2</sub> Si | SiF <sub>2</sub> Cl <sub>2</sub>                | Tetrafluormethylamin                                                                                         |            |        |             |
|                                   |                                                 | difluoro dichlorosilane                                                                                      | 18356-71-3 | 136.99 | -31.8       |
| ClF <sub>2</sub> HSi              | SiF <sub>2</sub> HCl                            | Difluor dichlorosilan (germ.)                                                                                |            |        |             |
|                                   |                                                 | difluoro chlorosilane                                                                                        | 80003-43-6 | 102.56 | -50.0       |
| ClF <sub>2</sub> P                | PF <sub>2</sub> Cl                              | Difluor dichlorosilan (germ.)                                                                                |            |        |             |
|                                   |                                                 | Phosphorus chloride                                                                                          | 14335-40-1 | 104.42 | -47.3       |
| ClF <sub>3</sub> Si               | SiClF <sub>3</sub>                              | difluoride                                                                                                   |            |        |             |
| ClH                               | HCl                                             | Chlorot trifluorosilane                                                                                      | 14049-36-6 | 120.53 | -70.2       |
| ClH <sub>3</sub> Si               | SiH <sub>3</sub> Cl                             | Hydrogen chloride                                                                                            | 7647-01-0  | 36.46  | -85.0       |
| CO                                | CO                                              | Chlorosilane                                                                                                 | 13465-78-6 | 66.56  | -30.3       |
| CO <sub>2</sub>                   | CO <sub>2</sub>                                 | Carbon monoxide                                                                                              | 630-08-0   | 28.01  | -191.5      |
| COS                               | OCS                                             | Carbon dioxide                                                                                               | 124-38-9   | 44.01  | -78.4       |
| F <sub>2</sub> HN                 | NHF <sub>2</sub>                                | Carbonyl sulfide                                                                                             | 463-58-1   | 60.07  | -50.3       |
| F <sub>2</sub> N <sub>2</sub>     | FNNF                                            | Difluoramine                                                                                                 | 10405-27-3 | 53.01  | -23.2       |
| F <sub>2</sub> N <sub>2</sub>     | FNNF                                            | trans-Difluorodiazine                                                                                        | 13776-62-0 | 66.01  | -111.5      |
| F <sub>2</sub> OS                 | F <sub>2</sub> SO                               | cis-Difluorodiazine                                                                                          | 13812-43-6 | 66.01  | -105.8      |
| F <sub>3</sub> HSi                | SiHF <sub>3</sub>                               | Thionyl fluoride                                                                                             | 7783-42-8  | 86.06  | -43.8       |
| F <sub>3</sub> N                  | NF <sub>3</sub>                                 | Trifluorosilane                                                                                              | 13465-71-9 | 86.09  | -95.2       |
| F <sub>3</sub> NO                 | NOF <sub>3</sub>                                | Nitrogen trifluoride                                                                                         | 7783-54-2  | 71.00  | -129.1      |
| F <sub>3</sub> NS                 | NSF <sub>3</sub>                                | Trifluoramine oxide                                                                                          | 13847-65-9 | 87.00  | -87.5       |
| F <sub>3</sub> P                  | PF <sub>3</sub>                                 | Thia zyl trifluoride                                                                                         | 15930-75-3 | 103.07 | -27.1       |
| F <sub>4</sub> Ge                 | GeF <sub>4</sub>                                | Phosphorus trifluoride                                                                                       | 7783-55-3  | 87.97  | -101.5      |
| F <sub>4</sub> Si                 | SiF <sub>4</sub>                                | Germanium(IV) fluoride                                                                                       | 7783-58-6  | 148.58 | -36.5       |
| F <sub>5</sub> P                  | PF <sub>5</sub>                                 | Tetrafluorosilane                                                                                            | 7783-61-1  | 104.08 | -86.0       |
| F <sub>6</sub> Se                 | SeF <sub>6</sub>                                | Phosphorus pentafluoride                                                                                     | 7647-19-0  | 125.97 | -84.5       |
| F <sub>6</sub> Te                 | TeF <sub>6</sub>                                | Selenium hexafluoride                                                                                        | 7783-79-1  | 192.95 | -46.5       |
| FH <sub>3</sub> Si                | SiH <sub>3</sub> F                              | Tellurium hexafluoride                                                                                       | 7783-80-4  | 241.59 | -38.8       |
| FNO                               |                                                 | fluorosilane                                                                                                 | 13537-33-2 | 50.11  | -98.0       |
| FNO <sub>3</sub>                  |                                                 | Nitrosyl fluoride                                                                                            | 7789-25-5  | 49.00  | -59.9       |
|                                   |                                                 | Fluorine nitrate                                                                                             | 7789-26-6  | 81.00  | -46.2       |

TABLE 1-continued

| Dielectric Compound | Structure | Name             | CAS        | MW     | MY BP(° C.) |
|---------------------|-----------|------------------|------------|--------|-------------|
| H2S                 | H2S       | Hydrogen sulfide | 7783-06-4  | 34.08  | -59.5       |
| H3N                 | NH3       | Ammonia          | 7664-41-7  | 17.03  | -33.3       |
| He                  | He        | Helium           | 7440-59-7  | 4.00   | -268.9      |
| HI                  | HI        | Hydrogen iodide  | 10034-85-2 | 127.91 | -35.6       |
| Kr                  | Kr        | Krypton          | 7439-90-9  | 83.80  | -153.4      |
| N2                  | N2        | Nitrogen         | 7727-37-9  | 28.01  | -195.8      |
| N2O                 | NNO       | dinitrogen oxide | 10024-97-2 | 44.01  | -88.5       |
| Ne                  | Ne        | Neon             | 7440-01-9  | 20.18  | -246.1      |
| NO                  | NO        | Nitrogen oxide   | 10102-43-9 | 30.01  | -151.8      |
| Xe                  | Xe        | Xenon            | 7440-63-3  | 131.29 | -108.1      |

15

The preferred dielectric compounds are selected from the group consisting of those set forth in Table 2 below:

TABLE 2

| Dielectric Compound | Structure  | Name                                                                                                                                   | CAS        | MW     | MY BP(° C.) |
|---------------------|------------|----------------------------------------------------------------------------------------------------------------------------------------|------------|--------|-------------|
| Ar                  | Ar         | Argon                                                                                                                                  | 7440-37-1  | 39.95  | -185.9      |
| BF3                 | BF3        | Trifluoroborane                                                                                                                        | 7637-07-2  | 67.81  | -101.2      |
| BrH                 | HBr        | Hydrogen bromide                                                                                                                       | 10035-10-6 | 80.91  | -66.7       |
| C2BrF5              | CF3CF2Br   | Bromopentafluoroethane                                                                                                                 | 354-55-2   | 198.92 | -21.0       |
| C2ClF3              | CFCl=CF2   | Chlorotrifluoroethene                                                                                                                  | 79-38-9    | 116.47 | -28.4       |
| C2F3N               | CF3CN      | Trifluoroacetonitrile                                                                                                                  | 353-85-5   | 95.02  | -68.8       |
| C2F3NO              | (CF3)NCO   | trifluoromethyl isocyanate                                                                                                             | 460-49-1   | 111.02 | -36.0       |
| C2F4S               | CF3C(S)F   | trifluoromethyl thiocarbonyl fluoride                                                                                                  | 132.08     | 21.0   |             |
|                     |            | Trifluoromethylthiocarbonylfluoride (germ.)                                                                                            |            |        |             |
| C2F5NO              | CF3CF2NO   | pentafluoro-nitroso-ethane//Pentafluor-nitroso-aethan                                                                                  | 354-72-3   | 149.02 | -45.7       |
| C2F5NO              | CF3C(O)NF2 | (trifluoromethyl-carbonyl)-difluoro-amine                                                                                              | 32822-49-4 | 149.02 | -21.1       |
| C2F6                | CF3CF3     | Hexafluoroethane                                                                                                                       | 76-16-4    | 138.01 | -78.2       |
| C2F6NO              | CF3N(O)CF3 | Bis-trifluoromethyl-nitroxid                                                                                                           | 2154-71-4  | 168.02 | -20.0       |
| C2F6O               | CF3OCF3    | bis-trifluoromethyl ether                                                                                                              | 1479-49-8  | 154.01 | -59.0       |
| C2F6Te              | (CF3)2Te   | bis(trifluoromethyl)tellurium                                                                                                          | 55642-42-7 | 265.61 | -98.0       |
| C2F6Te2             | CF3TeTeCF3 | bis(trifluoromethyl)ditelluride                                                                                                        | 1718-20-3  | 393.21 | -53.0       |
| C2F7N               | CF3CF2NF2  | N,N-Difluor-pentafluoroethylamin (germ.)                                                                                               | 354-80-3   | 171.02 | -38.0       |
| C2F7N               | (CF3)2NF   | N-Fluor-bis(trifluoromethyl)-amin (germ.)                                                                                              | 359-62-6   | 171.02 | -37.0       |
| C2F7NO              | CF3NFOCF3  | N-Fluor-N-trifluormethoxy-perfluoromethylamin (germ.)                                                                                  | 4217-92-9  | 187.02 | -25.0       |
| C2FNO               | FC(O)CN    | fluoroformyl cyanide                                                                                                                   | 683-55-6   | 73.03  | -21.0       |
| C2H2ClF             | CH2FCF1    | 1-chloro-1-fluoro-ethene//1-Chlor-1-fluor-aethen//1-chloro-1-fluoroethylene                                                            | 2317-91-1  | 80.49  | -25.5       |
| C2H2F2              | CF2=CH2    | 1,1-Difluoroethene                                                                                                                     | 75-38-7    | 64.03  | -85.7       |
| C2H2F2              | CHF=CHF    | #trans!-1,2-difluoro-ethene//#trans!-vinylene difluoride//(E)-1,2-difluoroethylene//(E)-1,2-difluoro-ethene//#trans!-vinylene fluoride | 1630-78-0  | 64.03  | -53.1       |
| C2H2F2              | FHC=CHF    | 1,2-difluoro-ethene//#cis!-vinylene difluoride//1,2-Difluor-aethen/vinylene fluoride                                                   | 1691-13-0  | 64.03  | -28.0       |
| C2H2F2              | CHF=CHF    | #cis!-1,2-difluoro-ethene//#cis!-vinylene difluoride//(Z)-1,2-difluoroethylene//(Z)-1,2-difluoro-ethene//#cis!-vinylene fluoride       | 1630-77-9  | 64.03  | -26.0       |
| C2H2F4              | CF3CH2F    | 1,1,1,2-Tetrafluoroethane                                                                                                              | 811-97-2   | 102.03 | -26.1       |
| C2H2F4              | CF2HCF2H   | 1,1,2,2-Tetrafluoroethane                                                                                                              | 359-35-3   | 102.03 | -23.0       |
| C2H3F               | CH2=CHF    | Fluoroethene                                                                                                                           | 75-02-5    | 46.04  | -72.2       |
| C2H3F3              | CF3CH3     | 1,1,1-Trifluoroethane                                                                                                                  | 420-46-2   | 84.04  | -47.3       |

TABLE 2-continued

| Dielectric Compound | Structure              | Name                                                                                             | CAS         | MW     | MY BP(° C.) |
|---------------------|------------------------|--------------------------------------------------------------------------------------------------|-------------|--------|-------------|
| C2H3F3O             | F3COCH3                | Ether, methyl trifluoromethyl                                                                    | 421-14-7    | 100.04 | -24.0       |
| C2H4                | H2CCH2                 | Ethene                                                                                           | 74-85-1     | 28.05  | -103.7      |
| C2H4F2              | CHF2CH3                | 1,1-Difluoroethane                                                                               | 75-37-6     | 66.05  | -24.0       |
| C2H5F               | CH3CH2F                | Fluoroethane                                                                                     | 353-36-6    | 48.06  | -37.7       |
| C2H6                | CH3CH3                 | Ethane                                                                                           | 74-84-0     | 30.07  | -88.6       |
| C2H6BF              | (CH3)2BF               | fluoro-dimethyl-borane                                                                           | 353-46-8    | 59.88  | -44.0       |
| C2H6F4OSi2          | CH3SiF2OSiF2CH3        | Disiloxane, 1,1,3,3-tetrafluoro-1,3-dimethyl-                                                    | 63089-45-2  | 178.23 | -39.0       |
| C2HF3               | CF2=CFH                | Trifluoroethene                                                                                  | 359-11-5    | 82.02  | -51.0       |
| C2HF3O              | CF3C(O)H               | trifluoroacetaldehyde//Trifluoracetaldehyd                                                       | 75-90-1     | 98.02  | -21.0       |
| C2HF5               | CF3CF2H                | Pentafluoroethane                                                                                | 354-33-6    | 120.02 | -48.1       |
| C2HF5O              | CF3OCHF2               | Difluoromethyl trifluoromethyl ether                                                             | 3822-68-2   | 136.02 | -35.3       |
| C3BiF9              | Bi(CF3)3               | Tris(trifluoromethyl)bismuth                                                                     | 5863-80-9   | 416.00 | -55.0       |
| C3F4                | F2C=C=CF2              | tetrafluoropropadiene//tetrafluoroallene//1,1,3,3-tetrafluoro-1,2-propadiene                     | 461-68-7    | 112.03 | -38.0       |
| C3F4                | =CFCF2CF=              | tetrafluorocyclopropene                                                                          | 19721-29-0  | 112.03 | -20.0       |
| C3F5IO              | CF3CF2(O)I             | Perfluoropropionyl iodid                                                                         | 137741-03-8 | 273.93 | -27.0       |
| C3F5N               | C2F5CN                 | pentafluoropropionitrile//pentafluoropropiononitrile                                             | 422-04-8    | 145.03 | -35.0       |
| C3F6                | cyclo<br>—CF2CF2CF2—   | hexafluorocyclopropane//Hexafluorocyclopropan//freon-#C1216                                      | 931-91-9    | 150.02 | -33.0       |
| C3F6                | CF3CF=CF2              | Hexafluoropropylene                                                                              | 116-15-4    | 150.02 | -29.6       |
| C3F6O2              | cyclo-CF2—O—CF2—CF2—O— | hexafluoro-[1,3]dioxolane                                                                        | 21297-65-4  | 182.02 | -22.1       |
| C3F8                | CF3CF2CF3              | Octafluoropropane                                                                                | 76-19-7     | 188.02 | -36.7       |
| C3F8O               | CF3CF2OCF3             | Perfluoromethyl ethylether                                                                       | 665-16-7    | 204.02 | -20.0       |
| C3H2F2              | F2CCH2                 | 1,1-difluoropropadiene//allenylidene difluoride//1,1-difluoroallene                              | 430-64-8    | 76.05  | -21.0       |
| C3H2F4              | H2CCFCF3               | 2,3,3,3-tetrafluoropropene//HFO-1234yf                                                           | 754-12-1    | 114.04 | -28.3       |
| C3H2F4              | CHF=CHCF3              | trans HFO-1234ze                                                                                 |             | 114.04 | -19.0       |
| C3H3F3              | CH2=CHCF3              | 3,3,3-Trifluoropropene                                                                           | 677-21-4    | 96.05  | -25.0       |
| C3H4                | c-(CH=CH—CH2)          | cyclopene                                                                                        | 2781-85-3   | 40.06  | -36.0       |
| C3H4                | H2CCH2                 | Allene                                                                                           | 463-49-0    | 40.06  | -34.5       |
| C3H4F2              | CH3CH=CF2              | 1,1-difluoropropene//propenylidene difluoride//1,1-Difluoropropene                               | 430-63-7    | 78.06  | -29.0       |
| C3H4O               |                        | methylketene                                                                                     | 6004-44-0   | 56.06  | -23.0       |
| C3H5F               | CH2CFCH3               | 2-fluoropropene                                                                                  | 1184-60-7   | 60.07  | -24.0       |
| C3H6                | CH2CHCH3               | 1-Propene                                                                                        | 115-07-1    | 42.08  | -47.7       |
| C3H7NO2             |                        | DL-2-aminopropanoic acid                                                                         | 302-72-7    | 89.09  | -50.2       |
| C3HF3               | F3CCCH                 | 3,3,3-trifluoropropyne//3,3,3-Trifluoropropin//trifluoromethyl-ethyne//3,3,3-trifluoro-1-propyne | 661-54-1    | 94.04  | -48.0       |
| C3HF5               | CF3CH=CF2              | 1,1,3,3,3-pentafluoropropene//1,1,3,3,3-Pentafluoropropene                                       | 690-27-7    | 132.03 | -21.0       |
| C3HF5               | CF3—CF—CFH             | 1,2,3,3,3-pentafluoropropene                                                                     | 2252-83-7   | 132.03 | -20.0       |
| C4F6                | CF3CCCCF3              | 1,1,1,4,4,4-hexafluoro-2-butyne                                                                  | 692-50-2    | 162.03 | -24.6       |
| C4H2F4O2            | CF2HC(O)C(O)CF2H       | 1,1,4,4-tetrafluoro-butane-2,3-dione                                                             |             | 158.05 | -81.0       |
| C4H6N2O2            |                        |                                                                                                  |             | 114.10 | -33.0       |
| CCIF3O              | F3C—O—Cl               | Trifluoromethylhypochlorit                                                                       | 22082-78-6  | 120.46 | -47.0       |
| CCIF3O              | ClF2C—OF               | Chlor-difluoromethylhypofluorit                                                                  | 20614-17-9  | 120.46 | -25.0       |
| CCIF4N              | CF3NFC1                | N-Chlor-N-fluorotrifluoromethylamin (gem.)                                                       | 13880-72-3  | 137.46 | -32.8       |
| CCIF4N              | C1CF2—NF2              | Chlordifluorodifluoraminomethan                                                                  | 13880-71-2  | 137.46 | -28.0       |
| CF2S                | F2C=S                  | thiocarbonyl difluoride                                                                          | 420-32-6    | 82.07  | -46.0       |
|                     |                        | (germ.)                                                                                          |             |        |             |
| CF2Se               | F2C=Se                 | selenocarbonyl difluoride                                                                        | 54393-39-4  | 128.97 | -28.0       |
| CF3I                | CF3I                   | Trifluoroiodomethane                                                                             | 2314-97-8   | 195.91 | -21.8       |
| CF3N                | CF2—N—F                | N-Fluor-difluormethanimin (germ.)                                                                | 338-66-9    | 83.01  | -101.0      |

TABLE 2-continued

| Dielectric Compound               | Structure                                       | Name                                                                                                        | CAS        | MW     | MY BP(° C.) |
|-----------------------------------|-------------------------------------------------|-------------------------------------------------------------------------------------------------------------|------------|--------|-------------|
| CF <sub>3</sub> NO                | CF <sub>3</sub> N=O                             | trifluoro-nitroso-methane//Trifluor-nitroso-methan                                                          | 334-99-6   | 99.01  | -86.0       |
| CF <sub>3</sub> NO                | FC(O)NF <sub>2</sub>                            | difluoro-carbamoyl fluoride                                                                                 | 2368-32-3  | 99.01  | -52.0       |
| CF <sub>3</sub> NO <sub>2</sub>   | CF <sub>3</sub> NO <sub>2</sub>                 | trifluoro-nitro-methane//Trifluor-nitro-methan//fluoropicrin                                                | 335-02-4   | 115.01 | -33.6       |
| CF <sub>4</sub>                   | CF <sub>4</sub>                                 | Tetrafluoromethane                                                                                          | 75-73-0    | 88.00  | -128.1      |
| CF <sub>4</sub> N <sub>2</sub>    | NF <sub>2</sub> CF=NF                           | Tetrafluorformamidin (gem.)                                                                                 | 14362-70-0 | 116.02 | -30.0       |
| CF <sub>4</sub> N <sub>2</sub> O  | (NF <sub>2</sub> ) <sub>2</sub> CO              | tetrafluorourea                                                                                             | 10256-92-5 | 132.02 | -20.0       |
| CF <sub>4</sub> O                 |                                                 | hypofluorous acid trifluoromethyl ester//Hypofluorigsaeure-trifluoromethylester/trifluoromethylhypofluorite |            | 104.00 | -95.0       |
| CF <sub>4</sub> O <sub>2</sub> S  | CF <sub>3</sub> SO <sub>2</sub> F               | trifluoromethanesulfonyl fluoride                                                                           | 335-05-7   | 152.07 | -21.7       |
| CF <sub>5</sub> N                 | CF <sub>3</sub> NF <sub>2</sub>                 | N,N-Difluor-trifluormethylamin (gem.)                                                                       | 335-01-3   | 121.01 | -75.0       |
| CF <sub>5</sub> NO                | CF <sub>3</sub> ONF <sub>2</sub>                | Trifluormethyloxidifluoramin (Difluoraminoxy)disfluoromethyl-hypofluorit                                    | 4217-93-0  | 137.01 | -59.8       |
| CF <sub>5</sub> NO <sub>2</sub>   | F <sub>2</sub> NOCF <sub>2</sub> OF             |                                                                                                             | 36781-60-9 | 153.01 | -29.0       |
| CF <sub>5</sub> NS                | SF <sub>5</sub> CN                              | sulfuryanide pentafluoride                                                                                  | 1512-13-6  | 153.08 | -25.0       |
| CF <sub>5</sub> P                 | CF <sub>3</sub> PF <sub>2</sub>                 | Schwefelcyanid-pentafluorid (germ.) difluoro-trifluoromethyl-phosphine                                      | 1112-04-5  | 137.98 | -43.0       |
| CF <sub>6</sub> N <sub>2</sub>    | F <sub>2</sub> NCF <sub>2</sub> NF <sub>2</sub> | Hexafluormethandiamin                                                                                       | 4394-93-8  | 154.01 | -37.0       |
| CF <sub>6</sub> Si                | CF <sub>3</sub> SiF <sub>3</sub>                | perfluoro methyl silane                                                                                     | 335-06-8   | 154.09 | -42.0       |
| CF <sub>7</sub> P                 | CF <sub>3</sub> PF <sub>4</sub>                 | Perfluormethylsilan (germ.) Trifluormethyl-tetrafluorophorran (germ.)                                       | 1184-81-2  | 175.97 | -35.0       |
| CH <sub>2</sub> F <sub>2</sub>    | CH <sub>2</sub> F <sub>2</sub>                  | Difluoromethane                                                                                             | 75-10-5    | 52.02  | -51.7       |
| CH <sub>2</sub> FI                | CH <sub>2</sub> FI                              | Fluoroiodomethane                                                                                           | 373-53-5   | 159.93 | -53.8       |
| CH <sub>3</sub> F                 |                                                 | fluoromethane//methyl fluoride//Fluormethan//freon-41                                                       | 593-53-3   | 34.03  | -78.3       |
| CH <sub>3</sub> F <sub>3</sub> Si | CF <sub>3</sub> SiH <sub>3</sub>                | trifluoromethyl-silane" CF <sub>3</sub> SiH <sub>3</sub>                                                    | 10112-11-5 | 100.12 | -38.3       |
| CH <sub>3</sub> F <sub>3</sub> Si | CH <sub>3</sub> SiF <sub>3</sub>                | methyltrifluorosilane                                                                                       | 373-74-0   | 100.12 | -30.0       |
| CH <sub>4</sub> F <sub>2</sub> Si | F <sub>2</sub> HSiCH <sub>3</sub>               | difluoro-methyl-silane                                                                                      | 420-34-8   | 82.12  | -35.6       |
| CH <sub>5</sub> FSi               | CH <sub>3</sub> SiH <sub>2</sub> F              | fluoro-methyl-silane                                                                                        | 753-44-6   | 64.13  | -44.0       |
| CH <sub>6</sub> Ge                | H <sub>3</sub> GeCH <sub>3</sub>                | methylgermane                                                                                               | 1449-65-6  | 90.65  | -23.0       |
| CHF <sub>2</sub> N                | F <sub>2</sub> C=NH                             | Difluorformimin                                                                                             | 2712-98-3  | 65.02  | -22.0       |
| CHF <sub>3</sub>                  | CHF <sub>3</sub>                                | Trifluoromethane                                                                                            | 75-46-7    | 70.01  | -82.1       |
| CHF <sub>3</sub> S                | CF <sub>3</sub> SH                              | trifluoromethane thiol                                                                                      | 1493-15-8  | 102.08 | -36.7       |
| CHF <sub>4</sub> N                | CF <sub>2</sub> H—NF <sub>2</sub>               | Trifluormethanthiol (germ.) N,N,1,1-Tetrafluormethylamin                                                    | 24708-53-0 | 103.02 | -43.0       |
| Cl <sub>2</sub> F <sub>2</sub> Si | SiF <sub>2</sub> Cl <sub>2</sub>                | difluoro dichlorosilane                                                                                     | 18356-71-3 | 136.99 | -31.8       |
| ClF <sub>2</sub> HSi              | SiF <sub>2</sub> HCl                            | Difluoridchlorsilan (germ.) difluoro chlorosilane                                                           | 80003-43-6 | 102.56 | -50.0       |
| ClF <sub>2</sub> P                | PF <sub>2</sub> Cl                              | Difluorchlorsilan (germ.) Phosphorus chloride difluoride                                                    | 14335-40-1 | 104.42 | -47.3       |
| ClF <sub>3</sub> Si               | SiClF <sub>3</sub>                              | Chlorotrifluorosilane                                                                                       | 14049-36-6 | 120.53 | -70.2       |
| ClH                               | HCl                                             | Hydrogen chloride                                                                                           | 7647-01-0  | 36.46  | -85.0       |
| ClH <sub>3</sub> Si               | SiH <sub>3</sub> Cl                             | Chlorosilane                                                                                                | 13465-78-6 | 66.56  | -30.3       |
| CO                                | CO                                              | Carbon monoxide                                                                                             | 630-08-0   | 28.01  | -191.5      |
| CO <sub>2</sub>                   | CO <sub>2</sub>                                 | Carbon dioxide                                                                                              | 124-38-9   | 44.01  | -78.4       |
| COS                               | OCS                                             | Carbonyl sulfide                                                                                            | 463-58-1   | 60.07  | -50.3       |
| F <sub>2</sub> HN                 | NHF <sub>2</sub>                                | Difluoramine                                                                                                | 10405-27-3 | 53.01  | -23.2       |
| F <sub>2</sub> N <sub>2</sub>     | FNNF                                            | trans-Difluorodiazine                                                                                       | 13776-62-0 | 66.01  | -111.5      |
| F <sub>2</sub> N <sub>2</sub>     | FNNF                                            | cis-Difluorodiazine                                                                                         | 13812-43-6 | 66.01  | -105.8      |
| F <sub>2</sub> OS                 | F <sub>2</sub> SO                               | Thionyl fluoride                                                                                            | 7783-42-8  | 86.06  | -43.8       |
| F <sub>3</sub> HSi                | SiHF <sub>3</sub>                               | Trifluorosilane                                                                                             | 13465-71-9 | 86.09  | -95.2       |
| F <sub>3</sub> N                  | NF <sub>3</sub>                                 | Nitrogen trifluoride                                                                                        | 7783-54-2  | 71.00  | -129.1      |
| F <sub>3</sub> NO                 | NOF <sub>3</sub>                                | Trifluoramine oxide                                                                                         | 13847-65-9 | 87.00  | -87.5       |
| F <sub>3</sub> NS                 | NSF <sub>3</sub>                                | thiazyl trifluoride                                                                                         | 15930-75-3 | 103.07 | -27.1       |
| F <sub>3</sub> P                  | PF <sub>3</sub>                                 | Phosphorus trifluoride                                                                                      | 7783-55-3  | 87.97  | -101.5      |
| F <sub>4</sub> Ge                 | GeF <sub>4</sub>                                | Germanium(IV) fluoride                                                                                      | 7783-58-6  | 148.58 | -36.5       |
| F <sub>4</sub> Si                 | SiF <sub>4</sub>                                | Tetrafluorosilane                                                                                           | 7783-61-1  | 104.08 | -86.0       |
| F <sub>5</sub> P                  | PF <sub>5</sub>                                 | Phosphorus pentafluoride                                                                                    | 7647-19-0  | 125.97 | -84.5       |
| F <sub>6</sub> Se                 | SeF <sub>6</sub>                                | Selenium hexafluoride                                                                                       | 7783-79-1  | 192.95 | -46.5       |
| F <sub>6</sub> Te                 | TeF <sub>6</sub>                                | Tellurium hexafluoride                                                                                      | 7783-80-4  | 241.59 | -38.8       |
| FH <sub>3</sub> Si                | SiH <sub>3</sub> F                              | fluorosilane                                                                                                | 13537-33-2 | 50.11  | -98.0       |

TABLE 2-continued

| Dielectric Compound | Structure        | Name              | CAS        | MW     | MY BP(° C.) |
|---------------------|------------------|-------------------|------------|--------|-------------|
| FNO                 |                  | Nitrosyl fluoride | 7789-25-5  | 49.00  | -59.9       |
| FNO <sub>3</sub>    |                  | Fluorine nitrate  | 7789-26-6  | 81.00  | -46.2       |
| H <sub>2</sub> S    | H <sub>2</sub> S | Hydrogen sulfide  | 7783-06-4  | 34.08  | -59.5       |
| H <sub>3</sub> N    | NH <sub>3</sub>  | Ammonia           | 7664-41-7  | 17.03  | -33.3       |
| He                  | He               | Helium            | 7440-59-7  | 4.00   | -268.9      |
| HI                  | HI               | Hydrogen iodide   | 10034-85-2 | 127.91 | -35.6       |
| Kr                  | Kr               | Krypton           | 7439-90-9  | 83.80  | -153.4      |
| N <sub>2</sub>      | N <sub>2</sub>   | Nitrogen          | 7727-37-9  | 28.01  | -195.8      |
| N <sub>2</sub> O    | NON              | Nitrous oxide     | 10024-97-2 | 44.01  | -88.5       |
| Ne                  | Ne               | Neon              | 7440-01-9  | 20.18  | -246.1      |
| NO                  | NO               | Nitrogen oxide    | 10102-43-9 | 30.01  | -151.8      |
| Xe                  | Xe               | Xenon             | 7440-63-3  | 131.29 | -108.1      |

The aforementioned dielectric compounds may be used in pure form, but can also be used as part of an azeotrope, or a mixture with an appropriate second gas, i.e., nitrogen, CO<sub>2</sub> or N<sub>2</sub>O.

Particularly preferred non-electrical properties for dielectric gases according to the present disclosure, include:

Non-liquefying, e.g., T<sub>boil</sub> less than -20° C.

Chemically stable—decomposition temperature must be higher than hot spot temperature in equipment, e.g., T<sub>dec</sub>=200° C., and gas should not decompose in partial discharge spark (approximately 1000° K)

Low environmental impact, i.e., little to no destruction of ozone layer ODP=0; and low global warming impact GWP less than SF<sub>6</sub>

Acceptably low toxicity of gas and discharge byproducts

Electrical equipment property requirements for dielectric gases according to the present disclosure, include:

Insulation specific criteria include a critical field of E<sub>cr</sub>, and no conducting decomposition products should be generated by discharge

Switching specific criteria include high critical field of E<sub>cr</sub>, arcing stability, i.e., a gas must recombine to original molecular structure after being decomposed in switching arc (Gibbs free energy of reaction is<0)

Specific thermal interruption performance, i.e., must be able to interrupt current flow at ac current zero

Arc erosion product from equipment and gas must not form conduction deposits

Low velocity of sound

#### EXAMPLE 1

Measurements of the dielectric strength of potential alternatives were determined using ASTM D2477 or obtained from literature. These measurements were performed at 1 atmosphere pressure across a 0.1 inch gap and at ambient temperature.

In the intended applications, the gas will not be at 1 atmosphere pressure but at a higher pressure. In this example 5 atmospheres pressure is used as a maximum pressure. If the gas liquefies at a lower pressure than that pressure was used. These gases have higher dielectric strengths and break down voltages than air. Using 5 atmospheres (73.5 psia) pressure as the upper pressure (rating of the equipment).

| Gas             | Dielectric strength<br>kV/0.1 inch gap | Pressure<br>(psia) | Breakdown voltage at<br>maximum pressure<br>(kV/0.1 inch gap) |
|-----------------|----------------------------------------|--------------------|---------------------------------------------------------------|
| Air             | 4.75                                   | 73.5               | 23.75                                                         |
| R143a           | 5.8                                    | 73.5               | 29                                                            |
| R152a           | 5.9                                    | 73.5               | 29.5                                                          |
| R125            | 6.4                                    | 73.5               | 32                                                            |
| R134a           | 6.6                                    | 73.5               | 33                                                            |
| R22             | 7.2                                    | 73.5               | 39.9                                                          |
| R124            | 10.4                                   | 55.5               | 39.3                                                          |
| SF <sub>6</sub> | 14.0                                   | 73.5               | 70                                                            |
| C318            | 16.0                                   | 45.3               | 49.3                                                          |
| R115            | 16.0                                   | 73.6               | 80                                                            |
| R114            | 17.0                                   | 31.1               | 36                                                            |

#### EXAMPLE 2

The dielectric strength of additional gases is measured at 1 atmosphere and at the maximum system pressure. Their breakdown voltages are found to be greater than air, which allows smaller gaps and therefore smaller equipment than would be needed if air was used. Here the measurements were performed on CTFE (Chlorotrifluoroethylene), HCl (hydrogen chloride) and SiF<sub>4</sub> (silicon tetrafluoride).

Having described the invention in detail by reference to the preferred embodiments and specific examples thereof, it will be apparent that modifications and variations are possible without departing from the spirit and scope of the disclosure and claims.

What is claimed is:

1. An insulation gas in electrical equipment, the insulation gas consisting of phosphorous pentafluoride and at least one gas selected from the group consisting of nitrogen, CO<sub>2</sub>, and N<sub>2</sub>O.

2. The insulation-gas according to claim 1, wherein said electrical equipment is selected from the group consisting of current-interruption equipment, gas-insulated transmission lines, gas-insulated transformers, and gas-insulated substations.

\* \* \* \* \*